



US005141835A

# United States Patent [19]

Kato et al.

[11] Patent Number: 5,141,835

[45] Date of Patent: Aug. 25, 1992

[54] LIQUID DEVELOPER FOR  
ELECTROSTATIC PHOTOGRAPHY

[75] Inventors: Eiichi Kato; Hideyuki Hattori, both  
of Shizuoka, Japan

[73] Assignee: Fuji Photo Film Co., Ltd., Kanagawa,  
Japan

[21] Appl. No.: 697,179

[22] Filed: May 8, 1991

[30] Foreign Application Priority Data

May 10, 1990 [JP] Japan ..... 2-118533  
Jul. 6, 1990 [JP] Japan ..... 2-177359  
Jul. 12, 1990 [JP] Japan ..... 2-182755

[51] Int. Cl.<sup>5</sup> ..... G03G 9/135

[52] U.S. Cl. ..... 430/115; 430/49;  
430/114

[58] Field of Search ..... 430/49, 114, 115

[56] References Cited

U.S. PATENT DOCUMENTS

4,983,486 1/1991 Kato et al. ..... 430/115  
5,035,972 7/1991 El-Sayed et al. ..... 430/114  
5,041,352 8/1991 Kato et al. ..... 430/115 X  
5,049,468 9/1991 Kato et al. ..... 430/114  
5,055,369 10/1991 Kato et al. ..... 430/114  
5,073,470 12/1991 Kato et al. ..... 430/115 X  
5,073,471 12/1991 Kato et al. ..... 430/115 X

FOREIGN PATENT DOCUMENTS

0333497 9/1989 European Pat. Off. .

0366491 5/1990 European Pat. Off. .

## OTHER PUBLICATIONS

Patent Abstracts of Japan, vol. 14, No. 289, Jun. 21,  
1990.

Patent Abstracts of Japan, vol. 14, No. 162, Mar. 29,  
1990.

Primary Examiner—Roland Martin  
Attorney, Agent, or Firm—Sughrue, Mion, Zinn,  
Macpeak & Seas

[57]

## ABSTRACT

A liquid developer for electrostatic photography is disclosed. The liquid developer comprises at least resin grains dispersed in a non-aqueous solvent having an electric resistance of at least 10<sup>9</sup> cm and a dielectric constant of not higher than 3.5, wherein the dispersed resin grains are copolymer resin grains obtained by polymerizing a solution containing (1) at least a mono-functional monomer (A) which is soluble in the above-described non-aqueous solvent but becomes insoluble therein by being polymerized, and, optionally, a monomer (C) represented by the formula (III) or a monomer (D) represented by the formula (IV), in the presence of a dispersion-stabilizing resin soluble in the non-aqueous solvent, which is a graft type copolymer. The liquid developer of the present invention is excellent in re-dispersibility, storability, stability, image-reproducibility, and fixability, and provide a master plate for offset printing having high printing durability.

8 Claims, No Drawings

## LIQUID DEVELOPER FOR ELECTROSTATIC PHOTOGRAPHY

### FIELD OF THE INVENTION

The present invention relates to a liquid developer for electrostatic photography, which comprises resin grains dispersed in a liquid carrier having an electric resistance of at least  $10^9 \Omega\text{cm}$  and a dielectric constant of not higher than 3.5, and more particularly to a liquid developer for electrostatic photography excellent in re-dispersibility, storability, stability, image-reproducibility, and fixability.

### BACKGROUND OF THE INVENTION

In general, a liquid developer for electrostatic photography is prepared by dispersing an inorganic or organic pigment or dye such as carbon black, nigrosine, phthalocyanine blue, etc., a natural or synthetic resin such as an alkyd resin, an acrylic resin, rosine, synthetic rubber, etc., in a liquid having a high electric insulating property and a low dielectric constant, such as a petroleum aliphatic hydrocarbon, etc., and further adding a polarity-controlling agent such as a metal soap, lecithin, linseed oil, a higher fatty acid, a vinyl pyrrolidone-containing polymer, etc., to the resulting dispersion.

In such a developer, the resin is dispersed in the form of insoluble latex grains having a grain size of from several nm to several hundred nm. In a conventional liquid developer, however, a soluble dispersion-stabilizing resin added to the liquid developer and the polarity-controlling agent are insufficiently bonded to the insoluble latex grains, thereby the soluble dispersion-stabilizing resin and the polarity-controlling agent are in a state of easily dispersing in the liquid carrier. Accordingly, there is a fault that when the liquid developer is stored for a long period of time or repeatedly used, the dispersion-stabilizing resin is split off from the insoluble latex grains, thereby the latex grains are precipitated, aggregated, and accumulated to make the polarity thereof indistinct. Also, since the latex grains once aggregated or accumulated are reluctant to re-disperse, the latex grains remain everywhere in the developing machine attached thereto, which results in causing stains of images formed and malfunctions of the developing machine, such as clogging of a liquid feed pump, etc.

For overcoming such defects, a means of chemically bonding the soluble dispersion-stabilizing resin and the insoluble latex grains is disclosed in U.S. Pat. No. 3,990,980. However, the liquid developer disclosed therein is still insufficient although the dispersion stability of the grains to the spontaneous precipitation may be improved to some extent. Also, when the liquid developer is actually used in a developing apparatus, the toner adhered to parts of the developing apparatus solidified to form a film and the toner grains thus solidified are reluctant to redisperse and are insufficient in re-dispersion stability for practical use, which causes the malfunction of the apparatus and staining of duplicated images.

In the method of producing resin grains described in aforesaid U.S. Pat. No. 3,990,980, there is a very severe restriction in the combination of a dispersion stabilizer to be used and monomer(s) being insolubilized for producing mono-dispersed latex grains having a narrow grain size distribution. Mostly, the resin grains produced by the above-described method are grains of a broad grain size distribution containing a large amount

of coarse grains or poly-dispersed grains having two or more different mean grain sizes. In the above-described method, it is difficult to obtain mono-dispersed resin grains having a narrow grain size distribution and having a desired grain size, and the method often results in the formation of large grains having a mean grain size of  $1 \mu\text{m}$  or more or very fine grains having a mean grain size of  $0.1 \mu\text{m}$  or smaller. Furthermore, there is also a problem that the dispersion stabilizer used must be prepared by an extremely complicated process which requires a long reaction time.

Furthermore, for overcoming the above-described defects, a method for improving the dispersibility, redispersibility and storage stability of resin grains by forming insoluble dispersed resin grains by copolymerizing a monomer being insolubilized with a monomer containing a long chain alkyl group or a monomer containing at least two polar groups as disclosed in JP-A-60-179751 and JP-A-62-151868 (the term "JP-A" as used herein means an "unexamined published Japanese patent application"). Also, a method for improving the dispersibility, redispersibility and storage stability of resin grains by forming insoluble dispersed resin grains by copolymerizing a monomer being insolubilized with a monomer containing a long chain alkyl group or a monomer containing at least two polar groups in the presence of a polymer utilizing a di-functional monomer or a polymer utilizing a macromolecular reaction is disclosed in JP-A-60-185963, JP-A-61-63855, JP-A-62-166362 and JP-A-63-66567.

On the other hand, an attempt has recently been made to print a large number of prints such as more than 5,000 prints using a master plate for offset printing by electrophotography, and, as a result of improvement particularly in the master plate, it has become possible to print more than 10,000 prints of large size. Also, a noticeable progress has recently been made in shortening the operation time in an electrophotomechanical system and an improvement of quickening a development-fix steps in the system has been made.

Also, the rationalization of an electrophotomechanical system has been greatly required and, practically, it has been attempted to prolong an interval of the maintenance time of a printing plate making machine. In this attempt, a liquid developer which can be used for a long period of time without being renewed has been required.

The dispersed resin grains produced by the methods disclosed in JP-A-60-179751, JP-A-62-151868, JP-A-62-166362 and JP-A-63-66567 yet show an unsatisfactory performance with respect to the dispersibility and redispersibility of the resin grains when the resin grains are used at a long interval of maintenance or the development speed is increased. Also, these resin grains show an unsatisfactory performance with respect to the dispersibility and re-dispersibility of the resin grains and the printing durability of plates obtained by the development with a liquid developer containing such resin grains when a large size master plate (e.g., a size larger than A-3) is processed.

In particular, there has been a problem in the improvement of re-dispersibility of the dispersed resin grains when the plate processing operation is improved by prolonging the interval of maintenance of the plate processing machine, or when the image quality of the reproduced image is improved in case of using a large

size plate-making machine for a large size master plate without causing stains of the developing machine.

### SUMMARY OF THE INVENTION

The present invention has been made for solving the above-described problems inherent to conventional electrophotographic liquid developers.

An object of the present invention is to provide a liquid developer excellent in dispersion stability, re-dispersibility, and fixing property in an electrophotomechanical system wherein development-fix steps are quickened and the interval of maintenance thereof is prolonged.

Another object of the present invention is to provide a liquid developer excellent in dispersion stability, re-dispersibility, and fixing property in an electrophotomechanical system wherein development-fix steps are quickened and master plates of large sizes are processed.

Still another object of the present invention is to provide a liquid developer capable of forming an offset printing master plate having excellent receptivity for printing ink and printing durability by an electrophotography.

A further object of the present invention is to provide a liquid developer suitable for various electrostatic photographies and various transfer systems in addition to the above-described uses.

A still further object of the present invention is to provide a liquid developer capable of being used for any liquid developer-using systems such as ink jet recording, cathode ray tube recording, and recording by pressure variation or electrostatic variation.

The above-described objects have been attained by the present invention as described hereinafter in detail.

That is, the present invention provides a liquid developer for electrostatic photography comprising at least resin grains dispersed in a non-aqueous solvent having an electric resistance of at least  $10^9 \Omega\text{cm}$  and a dielectric constant of not higher than 3.5, wherein the dispersed resin grains are polymer resin grains obtained by polymerizing a solution containing at least a mono-functional monomer (A) which is soluble in the above-described non-aqueous solvent but becomes insoluble therein by being polymerized, in the presence of a dispersion-stabilizing resin which is soluble in the non-aqueous solvent and which is a graft type copolymer formed from (1) at least one mono-functional macromonomer (M) having a weight average molecular weight of from  $1 \times 10^3$  to  $2 \times 10^4$  comprising an AB block copolymer having a polymerizable double bond bonded to the terminal of polymer main chain of the B block of said AB block copolymer, and (2) at least one monomer (B) represented by the following general formula (II), said AB block copolymer being composed of an A block comprising a polymer component containing at least one polar group selected from a phosphono group, a carboxy group, a sulfo group, a hydroxyl group, a formyl group, a carboxyamido group, a sulfoamido group, an amino group, and a



group (wherein  $\text{R}_{11}$  represents  $-\text{R}_{12}$  or  $-\text{OR}_{12}$  (wherein  $\text{R}_{12}$  represents a hydrocarbon group)) and/or a polymer component corresponding to the mono-func-

tional monomer (A) and a B block containing at least one polymerizable component represented by the following general formula (I):



wherein  $\text{V}_0$  represents  $-\text{COO}-$ ,  $-\text{OCO}-$ ,  $-(\text{CH}_2)_n\text{OCO}-$ ,  $-(\text{CH}_2)_m\text{COO}-$  (wherein  $\text{l}_1$  and  $\text{l}_2$  each represents an integer of from 1 to 3),  $-\text{O}-$ ,  $-\text{SO}_2-$ ,  $-\text{CO}-$ ,



$-\text{CONHCOO}-$ ,  $-\text{CONHCONH}-$  or



(wherein  $\text{R}_{13}$  represents a hydrogen atom or a hydrocarbon group),  $\text{R}_0$  represents a hydrocarbon group, and  $\text{a}_1$  and  $\text{a}_2$ , which may be the same or different, each represents a hydrogen atom, a halogen atom, a cyano group, a hydrocarbon group having from 1 to 8 carbon atoms,  $-\text{COOZ}_1$  or  $-\text{COO}-\text{Z}_1$  bonded via a hydrocarbon group (wherein  $\text{Z}_1$  represents a hydrocarbon group having from 1 to 22 carbon atoms);



wherein  $\text{V}_1$  represents  $-\text{COO}-$ ,  $-\text{OCO}-$ ,  $-(\text{CH}_2)_n\text{OCO}-$ ,  $-(\text{CH}_2)_m\text{COO}-$  (wherein  $\text{l}_3$  and  $\text{l}_4$  each represents an integer of from 1 to 3) or  $-\text{O}-$ ,  $\text{R}_1$  represents an aliphatic group having 8 or more carbon atoms, and  $\text{b}_1$  and  $\text{b}_2$ , which may be the same or different, each represents a hydrogen atom, a halogen atom or a hydrocarbon group having from 1 to 6 carbon atoms.

In a preferred embodiment of the present invention, the disperse resin grains contained in the liquid developer are produced by copolymerizing a solution containing at least one mono-functional monomer (A) and at least one monomer (C) represented by the formula (III) having at least two polar groups and/or polar linking groups hereinafter described in detail, or at least one monomer (D) represented by the formula (IV) having an aliphatic group having at least 8 carbon atoms hereinafter described in detail, in the presence of a dispersion-stabilizing resin.

### DETAILED DESCRIPTION OF THE INVENTION

Then, the liquid developer of the present invention is described in detail.

As the liquid carrier for the liquid developer of the present invention having an electric resistance of at least  $10^9 \Omega\text{cm}$  and a dielectric constant of not higher than 3.5, straight chain or branched aliphatic hydrocarbons, alicyclic hydrocarbons, aromatic hydrocarbons,

and halogen-substituted derivatives thereof can be used. Examples of liquid carrier include octane, isoctane, decane, isodecane, decalin, nonane, dodecane, isododecane, cyclohexane, cyclooctane, cyclodecane, benzene, toluene, xylene, mesitylene, Isopar E, Isopar G, Isopar H, Isopar L (Isopar: trade name of Exxon Co.), Shellsol 70, Shellsol 71 (Shellsol: trade name of Shell Oil Co.), Amsco OMS and Amsco 460 solvent (Amsco: trade name of American Mineral Spirits Co.). They may be used singly or as a combination thereof.

The non-aqueous dispersed resin grains (hereinafter, often referred to as "dispersion resin grains" or "latex grains") which are the most important constituting element in the present invention are resin grains produced by polymerizing (so-called polymerization granulation method), in a non-aqueous solvent, the above-described mono-functional monomer (A) and, optionally, the monomer (C) or (D), in the presence of a dispersion-stabilizing resin which is soluble in the non-aqueous solvent and which is a graft type copolymer.

As the non-aqueous solvent used in the present invention, any solvents miscible with the above-described liquid carrier for the liquid developer for electrostatic photography can be basically used in the present invention.

That is, the non-aqueous solvent used in the production of the dispersion resin grains may be any solvent miscible with the above-described liquid carrier, and preferably includes straight chain or branched aliphatic hydrocarbons, alicyclic hydrocarbons, aromatic hydrocarbons, and halogen-substituted derivatives thereof.

Specific examples thereof are hexane, octane, isoctane, decane, isodecane, decalin, nonane, dodecane, isododecane, and isoparaffin type petroleum solvents such as Isopar E, Isopar G, Isopar H, Isopar L, Shellsol 70, Shellsol 71, Amsco OMS, and Amsco 460. These solvents may be used singly or as a combination thereof.

Other solvents can be used together with the above-described organic solvents for the production of the non-aqueous dispersion resin grains, and examples thereof include alcohols (e.g., methanol, ethanol, propyl alcohol, butyl alcohol, and fluorinated alcohols), ketones (e.g., acetone, methyl ethyl ketone, and cyclohexanone), carboxylic acid esters (e.g., methyl acetate, ethyl acetate, propyl acetate, butyl acetate, methyl propionate, and ethyl propionate), ethers (e.g., diethyl ether, dipropyl ether, tetrahydrofuran, and dioxane), and halogenated hydrocarbons (e.g., methylene dichloride, chloroform, carbon tetrachloride, dichloroethane, and methylchloroform).

It is preferred that the non-aqueous solvents which are used as a mixture thereof are distilled off by heating or under a reduced pressure after completion of the polymerization granulation. However, even when the solvent is brought in the liquid developer as a latex grain dispersion, the solvent gives no problem if the liquid electric resistance of the liquid developer is in the range satisfying the requirement of at least  $10^9 \Omega\text{cm}$ .

In general, it is preferred that the same solvent as the liquid carrier is used in the step of forming the resin dispersion and, such solvents include straight chain or branched aliphatic hydrocarbons, alicyclic hydrocarbons, aromatic hydrocarbons, halogenated hydrocarbons, etc., as described above.

The monomers used for the production of the non-aqueous dispersed resin include a non-functional monomer (A) which is soluble in the non-aqueous solvent but becomes insoluble by being polymerized, and a mono-

mer (C) represented by the formula (III) which has at least two polar groups and/or polar linking groups, and which is polymerizable with the monomer (A), or a monomer (D) represented by the formula (IV) which contains an aliphatic group having 8 or more carbon atoms and which is copolymerizable with the monomer (A).

The mono-functional monomer (A) used in the present invention may be a monofunctional monomer which 10 is soluble in the non-aqueous solvent but becomes insoluble by being polymerized.

Practical examples of the monomer (A) include the monomers represented by the following formula (V);



wherein  $\text{U}_3$  represents  $-\text{COO}-$ ,  $-\text{OCO}-$ ,  $-\text{CH}_2\text{OCO}-$ ,  $-\text{CH}_2\text{COO}-$ ,  $-\text{O}-$ ,  $-\text{CONHCOO}-$ ,  $-\text{CONHOOCO}-$ ,  $-\text{SO}_2-$ ,



or



(wherein  $\text{D}_2$  represents a hydrogen atom or an aliphatic group having from 1 to 8 carbon atoms which may be substituted (e.g., methyl, ethyl, propyl, butyl, 2-chloroethyl, 2-bromoethyl, 2-cyanoethyl, 2-hydroxyethyl, benzyl, chlorobenzyl, methylbenzyl, methoxybenzyl, phenethyl, 3-phenylpropyl, dimethylbenzyl, fluorobenzyl, 2-methoxyethyl, and 3-methoxypropyl).

$\text{D}_1$  in the above formula (V) represents an aliphatic group having from 1 to 6 carbon atoms which may be substituted (e.g., methyl, ethyl, propyl, butyl, 2-chloroethyl, 2,2-dichloroethyl, 2,2,2-trifluoroethyl, 2-bromoethyl, 2-glycidylethyl, 2-hydroxyethyl, 2-hydroxypropyl, 2,3-dihydroxypropyl, 2-hydroxy-3-chloropropyl, 2-cyanoethyl, 3-cyanopropyl, 2-nitroethyl, 2-methoxyethyl, 2-methanesulfonylethyl, 2-ethoxyethyl, N,N-dimethylaminoethyl, N,N-diethylaminoethyl, trimethoxysilylpropyl, 3-bromopropyl, 4-hydroxybutyl, 2-furylethyl, 2-thienylethyl, 2-pyridylethyl, 2-morpholinoethyl, 2-carboxyethyl, 3-carboxypropyl, 4-carboxybutyl, 2-phosphoethyl, 3-sulfopropyl, 4-sulfonybutyl, 2-carboxyamidoethyl, 3-sulfoamidopropyl, 2-N-methylcarboxyamidoethyl, cyclopentyl, chlorocyclohexyl, and dichloroethyl).

In the above formula (V),  $f_1$  and  $f_2$ , which may be the same or different, each represents the same group as  $a_1$  or  $a_2$  in formula (I).

Specific examples of the monofunctional monomer (A) are vinyl esters or allyl esters of an aliphatic carboxylic acid having from 1 to 6 carbon atoms (e.g., acetic acid, propionic acid, butyric acid, monochloroacetic acid, and trifluoropropionic acid); alkyl esters or alkyl amides of an unsaturated carboxylic acid such as acrylic acid, methacrylic acid, crotonic acid, itaconic acid,

maleic acid, etc. (wherein the alkyl moiety has from 1 to 4 carbon atoms and may be substituted, and examples of the alkyl group are methyl, ethyl, propyl, butyl, 2-chloroethyl, 2-bromoethyl, 2-fluoroethyl, trifluoroethyl, 2-hydroxyethyl, 2-cyanoethyl, 2-nitroethyl, 2-methoxyethyl, 2-methanesulfonylethyl, 2-benzenesulfonylethyl, 2-(N,N-dimethylamino)ethyl, 2-(N,N-diethylamino)ethyl, 2-carboxyethyl, 2-phosphoethyl, 4-carboxybutyl, 3-sulforpropyl, 4-sulfobutyl, 3-chloropropyl, 2-hydroxy-3-chloropropyl, 2-furfurylethyl, 2-pyridinylethyl, 2-thienylethyl, trimethoxysilylpropyl, and 2-carboxyamidoethyl); styrene derivatives (e.g., styrene, vinyltoluene,  $\alpha$ -methylstyrene, vinylnaphthalene, chlorostyrene, dichlorostyrene, bromostyrene, vinylbenzenecarboxylic acid, vinylbenzenesulfonic acid, chloromethylstyrene, hydroxymethylstyrene, methoxymethylstyrene, N,N-dimethylaminomethylstyrene, vinylbenzenecarboxamide, and vinylbenzenesulfoamide); unsaturated carboxylic acids such as acrylic acid, methacrylic acid, crotonic acid, maleic acid, itaconic acid, etc.; cyclic anhydrides of maleic acid and itaconic acid; acrylonitrile; methacrylonitrile; and heterocyclic compounds having a polymerizable double bond (practically the compounds described in *Kobunshi (Macromolecular) Data Handbook (Foundation)*, pages 175-184, edited by Kobunshi Gakkai, published by Baihukan, 1986, such as, for example, N-vinylpyridine, N-vinylimidazole, N-vinylpyrrolidone, vinylthiophene, vinyltetrahydrofuran, vinyloxazoline, vinylthiazole, and N-vinylmorpholine).

The monomers (A) may be used singly or as a combination thereof.

According to a preferred embodiment of the present invention, the dispersion resin grains used in the present invention are obtained by polymerizing a solution containing at least one mono-functional monomer (A) and at least one monomer (C) having at least two polar groups and/or polar linking groups, in the presence of the above-described dispersion-stabilizing resin.

Specific examples of the monomer (C) having at least two polar groups and/or polar linking groups are monomers represented by following formula (III)



wherein  $U_1$  represents  $-\text{O}-$ ,  $-\text{COO}-$ ,  $-\text{OCO}-$ ,  
 $-\text{CH}_2\text{OCO}-$ ,  $-\text{SO}_2-$ ,  $-\text{CONH}-$ ,  $-\text{SO}_2\text{NH}-$ .



(wherein  $E_1$  represents a hydrocarbon group or has the same meaning as the linking group  $(A_1-B_1)(A_2-B_2)$ ;  $E_0$  in the above-described formula (III);  $E_0$  represents a hydrogen atom or a hydrocarbon group having from 1 to 18 carbon atoms, which may be substituted with a halogen atom,  $-\text{OH}$ ,  $-\text{CN}$ ,  $-\text{NH}_2$ ,  $-\text{COOH}$ ,  $-\text{SO}_3\text{H}$ , or  $-\text{PO}_3\text{H}_2$ ;  $B_1$  and  $B_2$ , which may be the same or different, each represents  $-\text{O}-$ ,  $-\text{S}-$ ,  $-\text{CO}-$ ,  $-\text{CO}_2-$ ,  $-\text{OCO}-$ ,  $-\text{SO}_2-$ ,



—NHCO<sub>2</sub>— or —NHCONH— (wherein E<sub>2</sub> has the same meaning as E<sub>0</sub> described above); A<sub>1</sub> and A<sub>2</sub>, which may be the same or different, each represents a hydrocarbon group having from 1 to 18 carbon atoms which may be substituted or may contain



(wherein  $B_3$  and  $B_4$ , which may be the same or different, have the same meaning as  $B_1$  and  $B_2$  described above;  $A_4$  represents a hydrocarbon group having from 1 to 18 carbon atoms, which may be substituted; and  $E_3$  has the same meaning as  $E_0$ ) in the main chain bond;  $d_1$  and  $d_2$ , which may be the same or different, each represents a hydrogen atom, a hydrocarbon group,  $—COO—E_4$  or  $—COO—E_4$  bonded via a hydrocarbon group (wherein  $E_4$  represents a hydrogen atom or a hydrocarbon group which may be substituted); and  $r$ ,  $s$  and  $t$ , which may be the same or different, each represents an integer of from 0 to 4, provided that  $r$ ,  $s$  and  $t$  cannot be 0 at the same time.

Then, the monomer (C) represented by formula (III) used in the present invention is described hereinafter in more detail.

In formula (III),  $U_1$  preferably represents  $-\text{O}-$ ,  $-\text{COO}-$ ,  $-\text{OCO}-$ ,  $-\text{CH}_2\text{OCO}-$ ,  $-\text{CONH}-$ , or



(wherein  $E_1$  represents preferably an alkyl group having from 1 to 16 carbon atoms which may be substituted, an alkenyl group having from 2 to 16 carbon atoms which may be substituted, an alicyclic group having from 5 to 18 carbon atoms which may be substituted, or has the same meaning as the linking group,  $A_1-B_1-A_2-B_2-E_0$  in formula (III)).

$E_0$  preferably represents a hydrogen atom or an aliphatic group having from 1 to 16 carbon atoms which may be substituted with a halogen atom (e.g., chlorine and bromine),  $-\text{OH}$ ,  $-\text{CN}$ , or  $-\text{COOH}$  (examples of the aliphatic group include an alkyl group, an alkenyl group, and an aralkyl group).

$B_1$  and  $B_2$ , which may be the same or different, each preferably represents  $-\text{O}-$ ,  $-\text{S}-$ ,  $-\text{CO}-$ ,  $-\text{COO}-$ ,  $-\text{OCO}-$ .



(wherein  $E_2$  each has the same meaning as  $E_0$  described above).

$A_1$  and  $A_2$ , which may be the same or different, each preferably represents a hydrocarbon group having from 1 to 12 carbon atoms (examples of the hydrocarbon group include an alkylene group, an alkenylene group, an arylene group and a cycloalkylene group) which may be substituted or may contain



(wherein B<sub>3</sub> and B<sub>4</sub>, which may be the same or different, have the same meaning as B<sub>1</sub> and B<sub>2</sub> described above; A<sub>4</sub> preferably represents an alkylene group having not more than 12 carbon atoms, an alkenylene group having not more than 12 carbon atoms, or an arylene group having not more than 12 carbon atoms, and each of these groups may be substituted; and E<sub>3</sub> has the same meaning as E<sub>0</sub> described above) in the main chain bond thereof.

d<sub>1</sub> and d<sub>2</sub>, which may be the same or different, each preferably represents a hydrogen atom, a methyl group, —COO—E<sub>4</sub>, or —CH<sub>2</sub>COO—E<sub>4</sub> (wherein E<sub>4</sub> preferably represents a hydrogen atom, an alkyl group having not more than 18 carbon atoms, an alkenyl group having not more than 18 carbon atoms, an aralkyl group having not more than 18 carbon atoms or a cycloalkyl group having not more than 18 carbon atoms).

r, s, and t, which may be the same or different, each preferably represents an integer of 0, 1, 2 or 3, provided that r, s and t cannot be 0 at the same time.

More preferably, in formula (III), U<sub>1</sub> represents —COO—, —CONH—, or



25

and d<sub>1</sub> and d<sub>2</sub>, which may be the same or different, each represents a hydrogen atom, a methyl group —COO—E<sub>4</sub>, or —CH<sub>2</sub>COO—E<sub>4</sub> (wherein E<sub>4</sub> represents more preferably an alkyl group having from 1 to 12 carbon atoms).

Further, specific examples of A<sub>1</sub> and A<sub>2</sub> are composed of an optional combination of atomic groups such as



35

(wherein E<sub>5</sub> and E<sub>6</sub> each represents a hydrogen atom, an alkyl group, or a halogen atom).



40

(wherein B<sub>3</sub>, B<sub>4</sub>, E<sub>3</sub>, A<sub>4</sub> and t have the same meaning as described above), etc.

Also, in the linking group



55

in the formula (III), it is preferred that the linkage main chain composed of U<sub>1</sub>, A<sub>1</sub>, B<sub>1</sub>, A<sub>2</sub>, B<sub>2</sub>, and E<sub>0</sub> has a total number of atoms of at least 8. In this case, when U<sub>1</sub> represents



65

and E<sub>1</sub> represents +A<sub>1</sub>—B<sub>1</sub>—A<sub>2</sub>—B<sub>2</sub>—E<sub>0</sub>, the linkage main chain composed by E<sub>1</sub> is included in the above-described linkage main chain. Furthermore, —B—

—A<sub>4</sub>—B<sub>4</sub>—E<sub>3</sub>, in the case where A<sub>1</sub> or A<sub>2</sub> represents a hydrocarbon group containing



in the main chain bond is also included in the above-described linkage main chain.

As to the number of atoms of the linkage main chain, when, for example, U<sub>1</sub> represents —COO— or —CONH—, the oxo group (=O) and the hydrogen atom are not included in the number of atoms but the carbon atom(s), ether-type oxygen atom, and nitrogen atom each constituting the linkage main chain are included in the number of atoms. Thus, the number of atoms of —COO— and —CONH— is counted as 2. Also, when, for example, E<sub>0</sub> represents —C<sub>9</sub>H<sub>19</sub>, the hydrogen atoms thereof are not included in the number of atoms and the carbon atoms are included therein. Thus, the number of atoms in this case is counted as 9.

Specific examples of the monomer (C) represented by formula (III) are illustrated below.



-continued



-continued

(III-10)

5



(III-11)

10



(III-12)

15



(III-13)

20



(III-14)

25



(III-15)

30



(III-16)

40



(III-17)

45



(III-19)

50

According to another preferred embodiment of the present invention, the dispersion resin grains used in the present invention are copolymer resin grains produced by copolymerizing a solution containing at least one mono-functional monomer (A) and at least one monomer (D) having an aliphatic group having 8 or more carbon atoms, in the presence of the above-described dispersion-stabilizing resin.

(III-20)

55

Specific examples of the monomer (D) containing an aliphatic group having 8 or more carbon atoms include monomers shown by the following formula (IV):

60



(III-21)

65

wherein  $\text{E}_7$  represents an aliphatic group having 8 or more carbon atoms;  $\text{U}_2$  represents  $-\text{COO}-$ ,  $-\text{CONH}-$ ,



(wherein  $E_8$  represents an aliphatic group),  $—OCO—$ ,  $—CH_2COO—$ , or  $—O—$ ; and  $e_1$  and  $e_2$ , which may be the same or different, each represents a hydrogen atom, an alkyl group,  $—COOE_9$ , or  $—CH_2COOE_9$  (wherein  $E_9$  represents an aliphatic group).

In formula (IV),  $E_7$  represents preferably an alkyl group having a total number of carbon atoms of 10 or more, which may be substituted, or an alkenyl group having a total number of carbon atoms of 10 or more and  $U_2$  preferably represents  $—COO—$ ,  $—CONH—$ ,



(wherein  $E_8$  preferably represents an aliphatic group having from 1 to 32 carbon atoms (examples of the aliphatic group are an alkyl group, an alkenyl group, or an aralkyl group),  $—OCO—$ ,  $—CH_2OCO—$  or  $—O—$ .

Also,  $e_1$  and  $e_2$ , which may be the same or different, each preferably represents a hydrogen atom, a methyl group,  $—COOE_9$ , or  $—CH_2COOE_9$  (wherein  $E_9$  preferably represents an aliphatic group having from 1 to 32 carbon atoms, for example, an alkyl group, an alkenyl group, an aralkyl group, or a cycloalkyl group).

In formula (IV), it is more preferable that  $U_2$  represents  $—COO—$ ,  $—CONH—$ , or



$e_1$  and  $e_2$ , which may be the same or different, each represents a hydrogen atom or a methyl group; and  $E_7$  has the same meaning as described above.

Specific examples of the monomer (C) shown by formula (IV) are unsaturated carboxylic acid esters having an aliphatic group of from 10 to 32 total carbon atoms (examples of the carboxylic acid are acrylic acid, methacrylic acid, crotonic acid, maleic acid, and itaconic acid, and examples of the aliphatic group are decyl, dodecyl, tridecyl, tetradecyl, hexadecyl, octadecyl, docosanyl, dodecanyl, hexadecanyl, oleyl, linoleyl, and docosanyl; the above aliphatic group may have a substituent such as a halogen atom, a hydroxy group, an amino group, an alkoxy group, etc., or may have a hetero atom such as oxygen, sulfur, nitrogen, etc. in the carbon-carbon bond of the main chain thereof); unsaturated carboxylic acid amides having an aliphatic group having from 10 to 32 carbon atoms (the unsaturated carboxylic acid and the aliphatic group are same as those described above on the esters); vinyl esters or allyl esters of a higher aliphatic acid (examples of the higher aliphatic acid are lauric acid, myristic acid, stearic acid, oleic acid, linoleic acid, and behenic acid); and vinyl ethers substituted with an aliphatic group having from 10 to 32 carbon atoms (the aliphatic group is the same as described above).

According to the above-described preferred embodiment of the present invention, the dispersion resin grains used in the present invention are composed of at least one kind of the monomer (A) and at least one kind of the monomer (C) or (D), and it is also important that the desired dispersion resin grains can be obtained if the resin synthesized from these monomers is insoluble in

the non-aqueous solvent. More practically, the proportion of the monomer (C) or (D) shown by the general formula (III) or (IV), respectively, is preferably from 0.1 to 20% by weight, and more preferably from 0.2 to 5 8% by weight based on the amount of the monomer (A). The molecular weight of the dispersion resin grains is preferably from  $1 \times 10^3$  to  $1 \times 10^6$ , and more preferably from  $1 \times 10^4$  to  $1 \times 10^6$ .

The dispersion-stabilizing resin used in the present invention is a graft type copolymer formed from (1) at least one mono-functional macromonomer (M) composed of a component of the AB block copolymer and (2) at least one monomer represented by the formula (II), and is characterized by being soluble in the above-described non-aqueous solvent.

In particular, in the graft moiety of the graft type copolymer, the block portion apart from the polymer main chain of the graft type copolymer (i.e., A block) is characterized by comprising a polymerizable component containing at least one polar group selected from the above described specific polar groups ( $—COOH$ ,  $—PO_3H_2$ ,  $—SO_3H$ ,  $—OH$ ,



30 a carboxyamido group, a sulfoamide group, a formyl group, an amino group and a cyclic acid anhydride-containing group) and/or a polymer component corresponding to the same monomer as the monomer (A) to be insolubilized.

35 The weight average molecular weight of the graft type copolymer is from  $1.5 \times 10^4$  to  $3 \times 10^5$ , preferably from  $2 \times 10^4$  to  $1 \times 10^5$ .

When the weight average molecular weight of the graft type copolymer is outside the range of from 40  $1.5 \times 10^4$  to  $3 \times 10^5$ , a mean grain size of the resin grains obtained by polymerization granulation becomes high or has a broad distribution thereby losing mono-dispersibility or causing aggregates.

45 The content of the mono-functional macromonomer (M) as a copolymerizable component used in forming in the graft type copolymer is from 1% to 60% by weight, preferably from 5% to 40% by weight. When the content is less than 1% by weight, a number of graft portion markedly decreases whereby the chemical structure of 50 the graft type copolymer becomes to be similar to that of conventional random copolymers and the effect of the present invention for improving the redispersibility of the resin grains is not obtained. On the other hand, when the content exceeds 60% by weight, the resulting copolymer does not have a sufficient copolymerizability with the monomer (B) represented by the formula (II).

55 Further, the content of the monomer (B) represented by the formula (II) as a copolymerizable component used in forming in the graft type copolymer is from 40 to 60 99% by weight, preferably from 60 to 95% by weight.

On the other hand, the mono-functional macromonomer (M) of the present invention which comes to be the graft portion of the graft type copolymer has a weight average molecular weight of from  $1 \times 10^3$  to 65  $2 \times 10^4$ , preferably from  $2 \times 10^3$  to  $1 \times 10^4$ . When the

weight average molecular weight is less than  $1 \times 10^3$ , the redispersibility of the resulting dispersed resin grains decreases, and, when it exceeds  $2 \times 10^4$ , the copolymerizability of the macromonomer (M) with the monomer (B) represented by the formula (II) decreases whereby the desirable graft type copolymer cannot be obtained.

As described above, since the graft type copolymer of the present invention is soluble in the above-described non-aqueous solvent, either of the polymer main chain thereof or the B block containing the repeating unit represented by the formula (I) in the graft portion, or both, contains a repeating unit which renders the graft type copolymer soluble in the non-aqueous solvent.

The graft type copolymer used in the present invention is described hereinafter in detail.

In the mono-functional macromonomer (M) which constitutes the graft type copolymer, the polymer components of the A block include a component containing a specific polar group and/or a component corresponding to the mono-functional monomer (A) to be insolubilized.

Specific examples of polar groups include a phosphono group, a carboxyl group, a hydroxyl group, a formyl group, a carboxyamido group, a sulfoamido group, an amino group, a



30

group and a cyclic acid anhydride-containing group.

In the polar group

$\text{R}_{11}$  represents  $-\text{R}_{12}$  or  $-\text{OR}_{12}$  wherein  $\text{R}_{12}$  represents a hydrocarbon group. Preferred examples of the hydrocarbon group include an aliphatic group having from 1 to 8 carbon atoms which may be substituted (e.g., methyl, ethyl, propyl, butyl, hexyl, octyl, 2-chloroethyl, 40 2-methoxyethyl, 3-ethoxypropyl, allyl, 1-propenyl, butenyl, cyclohexyl, benzyl, phenethyl, 3-phenylpropyl, methylbenzyl, chlorobenzyl, fluorobenzyl, and methoxybenzyl), or an aryl group which may be substituted (e.g., phenyl, tolyl, ethylphenyl, propylphenyl, 45 chlorophenyl, fluorophenyl, bromophenyl, chloromethylphenyl, dichlorophenyl, methoxyphenyl, cyanophenyl, acetamidophenyl, acetylphenyl, butoxy, and butoxyphenyl).

The monomer which derives the above-described 50 polymer component containing the specific polar group may be any vinyl type compound which is copolymerizable with a polymer component constituting another block component of the AB block copolymer of the present invention, i.e., the repeating unit represented by 55 the formula (I), and which contains a polar group. Examples of such monomers are described, e.g., in Kobunshi Gakkai (ed.), *Kobunshi Data Handbook (Kisohen)*, Baihukan (1986). Specific examples of these monomers include acrylic acid,  $\alpha$ - and/or  $\beta$ -substituted acrylic 60 acids (e.g.,  $\alpha$ -acetoxy,  $\alpha$ -acetoxymethyl,  $\alpha$ -(2-amino)ethyl,  $\alpha$ -chloro,  $\alpha$ -bromo,  $\alpha$ -fluoro,  $\alpha$ -tributylsilyl,  $\alpha$ -cyano,  $\beta$ -chloro,  $\beta$ -bromo,  $\alpha$ -chloro- $\beta$ -methoxy, and  $\alpha$ , $\beta$ -dichloro compounds), methacrylic acid, itaconic acid, itaconic half esters, itaconic half amides, 65 crotonic acid, 2-alkenylcarboxylic acids (e.g., 2-pentenoic acid, 2-methyl-2-hexenoic acid, 2-octenoic acid, 4-methyl-2-hexenoic acid, and 4-ethyl-2-octenoic acid),

maleic acid, maleic half esters, maleic half amides, vinylbenzenecarboxylic acid, vinylbenzenesulfonic acid, vinylsulfonic acid, vinylphosphonic acid, dicarboxylic acid vinyl or allyl half esters, and ester or amide derivatives of these carboxylic acids or sulfonic acids containing the polar group in the substituent thereof.

Specific examples of these compounds are set forth below, but the present invention should not be construed as being limited thereto. In the following formulae, e represents  $-\text{H}$ ,  $-\text{CH}_3$ ,  $-\text{Cl}$ ,  $-\text{Br}$ ,  $-\text{CN}$ ,  $-\text{CH}_2\text{COOCH}_3$  or  $-\text{CH}_2\text{COOH}$ , f represents  $-\text{H}$  or  $-\text{CH}_3$ ,  $n_1$  represents an integer of 2 to 18,  $m_1$  represents an integer of 1 to 12, and  $l_1$  represents an integer of 1 to 4.





-continued



-continued



25 The polymer components which constitute the A block may be a polymer component corresponding to the monomer (A) to be insolubilized, in addition to the above-described polymer component containing the specific polar group. Specific examples of the polymer component include those corresponding to the above-described mono-functional monomer (A).

The B block of the polymer component comprises a repeating unit represented by the formula (I):

(41) (42) In the general formula (I),  $\text{V}_0$  represents  $-\text{COO}-$ ,  
 35  $-\text{OCO}-$ ,  $-\text{CH}_2\text{OOCO}-$ ,  $-\text{CH}_2\text{COO}-$  (wherein  $\text{l}_1$  and  $\text{l}_2$  each represents an integer of from 1 to 3),  
 $-\text{O}-$ ,  $-\text{SO}_2-$ ,  $-\text{CO}-$ ,

(43) (44) 40  $\text{R}_{13}$   $\text{R}_{13}$   
 $-\text{CON}-$ ,  $-\text{SO}_2\text{N}-$ ,

$-\text{CONHCOO}-$ ,  $-\text{CONHCONH}-$ , or



(45) 50 (wherein  $\text{R}_{13}$  represents a hydrogen atom or a hydrocarbon group).

Preferred examples of the hydrocarbon group represented by  $\text{R}_{13}$  include an alkyl group having from 1 to 18 carbon atoms which may be substituted (e.g., methyl, ethyl, propyl, butyl, pentyl, hexyl, heptyl octyl, decyl, dodecyl, hexadecyl, octadecyl, 2-chloroethyl, 2-bromoethyl, 2-cyanoethyl, 2-methoxycarbonylethyl, 2-methoxyethyl, and 3-bromopropyl), an alkenyl group having from 4 to 18 carbon atoms which may be substituted (e.g., 2-methyl-1-porpenyl, 2-butenyl, 2-pentenyl, 3-methyl-2-pentenyl, 1-pentenyl, 1-hexenyl, 2-hexenyl, and 4-methyl-2-hexenyl), an aralkyl group having from 7 to 12 carbon atoms which may be substituted (e.g., benzyl, phenethyl, 3-phenylpropyl, naphthylmethyl, 2-naphthylethyl, chlorobenzyl, bromobenzyl, methylbenzyl, ethylbenzyl, methoxybenzyl, dimethylbenzyl, and dimethoxybenzyl), an alicyclic group having from 5 to 8 carbon atoms which may be substituted (e.g., cyclo-

hexyl, 2-cyclohexylethyl, and 2-cyclopentylethyl), and an aromatic group having from 6 to 12 carbon atoms which may be substituted (e.g., phenyl, naphthyl, tolyl, xylol, propylphenyl, butylphenyl, octylphenyl, dodecylphenyl, methoxyphenyl, ethoxyphenyl, butoxyphenyl, decyloxyphenyl, chlorophenyl, dichlorophenyl, bromophenyl, cyanophenyl, acetylphenyl, methoxycarbonylphenyl, ethoxycarbonylphenyl, butoxycarbonylphenyl, acetamidophenyl, propioamidophenyl, and dodecyloylamidophenyl).

When  $V_0$  represents



the benzene ring may be substituted. Suitable examples of the substituents include a halogen atom (e.g., chlorine, and bromine), an alkyl group (e.g., methyl, ethyl, propyl, butyl, chloromethyl, and methoxymethyl), and an alkoxy group (e.g., methoxy, ethoxy, propoxy, and butoxy).

$R_0$  represents a hydrocarbon group, and preferred examples of the hydrocarbon group include an alkyl group having 1 to 22 carbon atoms which may be substituted (e.g., methyl, ethyl, propyl, butyl, heptyl, hexyl, octyl, decyl, dodecyl, tridecyl, tetradecyl, hexadecyl, octadecyl, 2-chloroethyl, 2-bromoethyl, 2-cyanoethyl, 30 2-methoxycarbonylethyl, 2-methoxyethyl, and 3-bromopropyl), an alkenyl group having from 4 to 18 carbon atoms (e.g., 2-methyl-1-propenyl, 2-butenyl, 2-pentenyl, 3-methyl-2-pentenyl, 1-pentenyl, 1-hexenyl, 2-hexenyl, and 4-methyl-2-hexenyl), an aralkyl group 35 having from 7 to 12 carbon atoms which may be substituted (e.g., benzyl, phenetyl, 3-phenylpropyl, naphthylmethyl, 2-naphthylethyl, chlorobenzyl, bromobenzyl, methylbenzyl, ethylbenzyl, methoxybenzyl, dimethylbenzyl, and dimethoxybenzyl), an alicyclic group having from 5 to 8 carbon atoms which may be substituted (e.g., cyclohexyl, 2-cyclohexylethyl, and 2-cyclopentylethyl), an aromatic group having from 6 to 12 carbon atoms which may be substituted (e.g., phenyl, naphthyl, tolyl, xylol, propylphenyl, butylphenyl, octylphenyl, dodecylphenyl, methoxyphenyl, ethoxyphenyl, butoxyphenyl, decyloxyphenyl, chlorophenyl, dichlorophenyl, bromophenyl, cyanophenyl, acetylphenyl, methoxycarbonylphenyl, ethoxycarbonylphenyl, butoxycarbonylphenyl, acetamidophenyl, propioamidophenyl, and dodecyloylamidophenyl).

In the general formula (I),  $a_1$  and  $a_2$ , which may be the same or different, each preferably represents a hydrogen atom, a halogen atom (e.g., chlorine, and bromine), a cyano group, an alkyl group having from 1 to 4 carbon atoms (e.g., methyl, ethyl, propyl, and butyl),  $-COO-Z_1$  or  $-COO-Z_1$  bonded via a hydrocarbon group, wherein  $Z_1$  represents a hydrocarbon group (preferably an alkyl group having 1 to 18 carbon atoms, an alkenyl group having 4 to 18 carbon atoms, an aralkyl group having 7 to 12 carbon atoms, an alicyclic group having 5 to 8 carbon atoms or an aryl group having 6 to 12 carbon atoms, each of which may be substituted). More specifically, the examples of the hydrocarbon groups are those described for  $R_{13}$  above. The hydrocarbon group via which  $-COO-Z_1$  is bonded includes, for example, a methylene group, an ethylene group, an a propylene group.

More preferably, in the general formula (I),  $V_0$  represents  $-COO-$ ,  $-OCO-$ ,  $-CH_2OCO-$ ,  $-CH_2COO-$ ,  $-O-$ ,  $-CONH-$ ,  $-SO_2NH-$  or



10 and  $a_1$  and  $a_2$ , which may be the same or different, each represents a hydrogen atom, a methyl group,  $-COOZ_1$ , or  $-CH_2COOZ_1$ , wherein  $Z_1$  represents an alkyl group having from 1 to 6 carbon atoms (e.g., methyl, ethyl, propyl, butyl, and hexyl). Most preferably, either one of  $a_1$  and  $a_2$  represents a hydrogen atom.

15 As the polymerizable component other than the repeating units represented by the general formula (I) which is contained in the B block together with the polymerizable component(s) selected from the repeating units of the general formula (I), any components copolymerizable with the repeating units of the general formula (I) can be used.

20 Suitable examples of monomers corresponding to the repeating unit copolymerizable with the polymerizable component represented by the general formula (I), as a polymerizable component in the B block include acrylonitrile, methacrylonitrile and heterocyclic vinyl compounds (e.g., vinylpyridine, vinylimidazole, vinylpyrrolidone, vinylthiophene, vinylpyrazole, vinyldioxane, and vinyloxazine). Such other monomers are employed in a range of not more than 20 parts by weight per 100 parts by weight of the total polymerizable components in the B block.

25 Further, it is preferred that the B block does not contain the polymerizable component containing a polar group which is a component constituting the A block.

30 In the mono-functional macromonomer (M) used in the graft type copolymer of the present invention, the proportion of the A block and the B block in the AB block copolymer is preferably 1 to 50/99 to 50 (weight ratio).

35 The content of the polymer component having a specific polar group contained in the A block is preferably from 1 to 30 parts by weight, more preferably from 1 to 15 parts by weight, per 100 parts by weight of the dispersion-stabilizing resin.

40 As described above, the macromonomer (M) to be used in the present invention has a structure of the AB block copolymer in which a polymerizable double bond group is bonded to one of the terminals of the B block composed of the polymerizable component represented by the general formula (I) and the other terminal thereof is connected to the A block composed of the polymerizable component containing the polar group or the polymerizable component corresponding to the mono-functional monomer (A). The polymerizable double bond group will be described in detail below.

45 Suitable examples of the polymerizable double bond group include those represented by the following general formula (VI):



wherein  $V_2$  has the same meaning as  $V_0$  defined in the general formula (I), and  $g_1$  and  $g_2$ , which may be the same or different, each has the same meaning as  $a_1$  and  $a_2$  defined in the general formula (I).

Specific examples of the polymerizable double bond group represented by the general formula (VI) include



The macromonomer (M) used in the present invention has a structure in which a polymerizable double bond group preferably represented by the general formula (VI) is bonded to one of the terminals of the B block either directly or through an appropriate linking group.

The linking group which can be used includes a carbon-carbon bond (either single bond or double bond), a carbon-hetero atom bond (the hetero atom includes, for example, an oxygen atom, a sulfur atom, a nitrogen atom, and a silicon atom), a hetero atom-hetero atom bond, and an appropriate combination thereof.

More specifically, the bond between the group of the general formula (VI) and the terminal of the B block is a mere bond or a linking group selected from



5

(wherein R<sub>14</sub> and R<sub>15</sub> each represents a hydrogen atom, a halogen atom (e.g., fluorine, chlorine, and bromine), a cyano group, a hydroxyl group, or an alkyl group (e.g., methyl, ethyl, and propyl),  $\text{--CH=CH--}$ ,



(wherein  $R_{16}$  and  $R_{17}$  each represents a hydrogen atom or a hydrocarbon group having the same meaning as defined for  $R_0$  in the general formula (I) described above), and an appropriate combination thereof.

If the weight average molecular weight of the macromonomer (M) exceeds  $2 \times 10^4$ , copolymerizability with monomer (B) is undesirably reduced. If, on the other hand, it is too small, the effect of improving electrophotographic characteristics of the light-sensitive layer would be small. Accordingly, the macromonomer (M) preferably has a weight average molecular weight of at least  $1 \times 10^3$ .

The macromonomer (M) used in the present invention can be produced by a conventionally known synthesis method. More specifically, it can be produced by the method comprising previously protecting the polar group of a monomer corresponding to the polymerizable component having the specific polar group to form a functional group, synthesizing an AB block copolymer 45 by a so-called known living polymerization reaction, for example, an ion polymerization reaction with an organic metal compound (e.g., alkyl lithiums, lithium diisopropylamide, and alkylmagnesium halides) or a 50 hydrogen iodide/iodine system, a photopolymerization reaction using a porphyrin metal complex as a catalyst, or a group transfer polymerization reaction, introducing a polymerizable double bond-containing group into the terminal of the resulting living polymer by a reaction 55 with a various kind of reagent, and then conducting a protection-removing reaction of the functional group which has been formed by protecting the polar group by a hydrolysis reaction, a hydrogenolysis reaction, an 60 oxidative decomposition reaction, or a photodecomposition reaction to form the polar group.

An example thereof is shown by the following reaction scheme (1):

Reaction Scheme (2)



The living polymer can be easily synthesized according to synthesis methods as described, e.g., in P. Lutz, P. Masson et al, *Polym. Bull.*, 12, 79 (1984), B. C. Anderson, G. D. Andrews et al, *Macromolecules*, 14, 1601 (1981), K. Hatada, K. Ute et al, *Polym. J.*, 17, 977 (1985), *ibid.*, 18, 1037 (1986), Koichi Migite and Koichi Hatada, *Kobunshi Kako (Polymer Processing)*, 36, 366 (1987), Toshinobu Higashimura and Mitsuo Sawamoto, *Kobunshi Ronbun Shu (Polymer Treatises)*, 46, 189 (1989), M. Kuroki and T. Aida, *J. Am. Chem. Soc.*, 109, 4737 (1987), Teizo Aida and Shohei Inoue, *Yuki Gosei Kagaku (Organic Synthesis Chemistry)*, 43, 300 (1985),

and D. Y. Sogoh, W. R. Hertler et al, *Macromolecules*, 20, 1473 (1987).

In order to introduce a polymerizable double bond-containing group into the terminal of the living polymer, a conventionally known synthesis method for macromonomer can be employed.

For details, reference can be made, for example, to P. Dreyfuss and R. P. Quirk, *Encycl. Polym. Sci. Eng.*, 7, 551 (1987), P. F. Rempp and E. Franta, *Adv. Polym. Sci.*, 58, 1 (1984), V. Percec, *Appl. Polym. Sci.*, 285, 95 (1984), R. Asami and M. Takari, *Makromol. Chem. Suppl.*, 12, 163 (1985), P. Rempp et al., *Makromol. Chem. Suppl.*, 8, 3 (1984), Yushi Kawakami, *Kogaku Kogyo*, 38, 56 (1987),

Yuya Yamashita, *Kobunshi*, 31, 988 (1982), Shiro Kobayashi, *Kobunshi*, 30, 625 (1981), Toshinobu Higashimura, *Nippon Sechaku Kyokaishi*, 18, 536 (1982), Koichi Itoh, *Kobunshi Kako*, 35, 262 (1986), Kishiro Higashi and Takashi Tsuda, *Kino Zairyo*, 1987, No. 10, 5, and references cited in these literatures.

Also, the protection of the specific polar group of the present invention and the release of the protective group (a reaction for removing a protective group) can be easily conducted by utilizing conventionally known techniques. More specifically, they can be performed by appropriately selecting methods as described, e.g., in Yoshio Iwakura and Keisuke Kurita, *Hannsei Kobunshi (Reactive Polymer)*, published by Kodansha (1977), T. W. Greene, *Protective Groups in Organic Synthesis*, published by John Wiley & Sons (1981), and J. F. W. McOmie, *Protective Groups in Organic Chemistry*, Plenum Press, (1973), as well as methods as described in the above references.

Furthermore, the AB block copolymer can be also synthesized by a photoinitiator polymerization method using a dithiocarbamate compound as photoinitiator. For example, the block copolymer can be synthesized according to synthesis methods as described, e.g., in Takayuki Otsu, *Kobunshi (Polymer)*, 37, 248 (1988), or or Shunichi Himori and Ryuichi Ohtsu, *Polym. Rep. Jap.* 37, 3508 (1988), JP-A-64-111, and JP-A-64-26619.

The macromonomer (M) according to the present invention can be obtained by applying the above described synthesis method for macromonomer to the AB block copolymer.

Specific examples of the macromonomer (M) which can be used in the present invention are set forth below, but the present invention should not be construed as being limited thereto. In the following formulae,  $a_1$ ,  $a_2$  and  $a_3$  each represents  $-H$ ,  $-CH_3$  or  $-CH_2COOCH_3$ ; R represents  $-C_nH_{2n+1}$  (wherein n represents an integer of from 1 to 18),



(wherein q represents an integer of from 1 to 3),

45



(wherein X represents  $-H$ ,  $-Cl$ ,  $-Br$ ,  $-CH_3$ ,  $-OCH_3$  or  $-COCH_3$ ) or



(wherein p represents an integer of from 0 to 3); l represents an integer of from 2 to 12;  $a_4$  represents  $-H$  or  $-CH_3$ ; Y represents  $-OH$ ,  $-COOH$ ,  $-SO_3H$ ,



$Y_1$  represents  $-COOH$ ,  $-SO_3H$ ,



$R'$  represents  $-C_mH_{2m+1}$  (wherein m represents an integer of from 1 to 8) or



(wherein q represents an integer of 1 to 3); k represents an integer of from 2 to 6; and  $-b-$  represents a block bond as defined above.



-continued



(M-3)



(M-4)



(M-5)



(M-6)



(M-7)



(M-8)



(M-9)



(M-10)

-continued

(M-11)



(M-12)



(M-13)



(M-14)



(M-15)



(M-16)



The dispersion-stabilizing resin used in the present invention is a graft type copolymer formed from at least one mono-functional macromonomer (M) and a monomer (B) represented by formula (II).

In formula (II), V<sub>1</sub> preferably represents —COO—, —OCO— or —O—.

R<sub>1</sub> represent an aliphatic group having 8 or more carbon atoms, preferably an alkyl group or an alkenyl group, each having 10 or more carbon atoms, which may be a straight chain or branched group. Specific examples of R<sub>1</sub> include decyl, dodecyl, tridecyl, tetradecyl, hexadecyl, octadecyl, eicosanyl, docosanyl, decenyl, dodecenyl, tridecenyl, hexadecenyl, octadecenyl, and linolenyl.

b<sub>1</sub> and b<sub>2</sub>, which may be the same or different, each preferably represents a hydrogen atom, a halogen atom or a hydrocarbon group having from 1 to 3 carbon atoms, and specific examples thereof include a hydrogen atom, a chlorine atom, a bromine atom, a methyl group, an ethyl group and a propyl group.

The proportion of the monomer selected from the monomers represented by formula (II) as a copolymer-

50 izable component used in forming in the above-described graft type copolymer is from 40 to 99 parts by weight, preferably from 60 to 95 parts by weight, per 100 parts by weight of the graft type copolymer.

55 Further, in addition to the macromonomer (M) and the monomer (B) of formula (II), the graft type copolymer used in the present invention may be formed from other monomers which are copolymerizable with the macromonomer (M) and the monomer (B) of formula (II), as a polymer component of the graft type copolymer. The proportion of such other monomers is 20% by weight or less, preferably 15% by weight or less, based on the weight of the graft type copolymer.

60 The dispersion resin grains (latex grains) used in the present invention can be generally produced by heat-polymerizing the above-described dispersion-stabilizing resin, the monomer (A) and, optionally, the monomer (C) or (D), in a non-aqueous solvent in the presence of a polymerization initiator such as benzoyl peroxide, azobis-isobutyronitrile, butyl-lithium, etc.

Practically, the dispersion resin grains can be produced by (1) a method of adding the polymerization initiator to a solution of a mixture of the dispersion-stabilizing resin, the monomer (A), and, optionally, the monomer (C) or (D), (2) a method of adding dropwise the monomer (A), and, optionally, the monomer (C) or (D), together with the polymerization initiator to a solution of the dispersion-stabilizing resin, (3) a method of adding the polymerization initiator and a part of a mixture of the monomer (A) and, optionally, the monomer (C) or (D) to a solution of the total amount of the dispersion-stabilizing resin and the remaining monomer (A) and, optionally, monomer (C) or (D), or (4) a method of adding a solution of the dispersion-stabilizing resin and the monomers (A) and, optionally, (C) or (D) together with the polymerization initiator to a non-aqueous solvent.

The total amount of the monomer (A) and, optionally, the monomer (C) or (D) is from about 5 to 80 parts by weight, and preferably from 10 to 50 parts by weight per 100 parts by weight of the non-aqueous solvent.

Also, the amount of the dispersion-stabilizing resin which is a soluble resin is from 1 to 100 parts by weight, and preferably from 3 to 50 parts by weight per 100 parts by weight of the monomer (A) or per 100 parts by weight of the total amounts of monomer (A) and monomer (C) or (D).

A suitable amount of the polymerization initiator is from 0.1 to 5% by weight of the total amount of monomer (A) or the monomers (A) and (C) or (D).

The polymerization temperature is from about 50° C. to 180° C., and preferably from 60° C. to 120° C. The reaction time is preferably from 1 to 15 hours.

When a polar solvent such as alcohols, ketones, ethers, esters, etc., is used together with the non-aqueous solvent for the above-described reaction or when unreacted monomer (A) and/or monomer (C) or (D) remain without being polymerization-granulated, it is preferred to distil off the polar solvent or the unreacted monomers by heating the reaction mixture to the boiling point of the solvent or the monomers or to remove the solvent or the monomers by distillation under reduced pressure.

The latex grains dispersed in a non-aqueous solvent thus produced exist as fine grains having a uniform grain size distribution and show a very stable dispersibility. In particular, when the liquid developer composed of the latex grains are repeatedly used in a developing device for a long period of time, the dispersibility thereof is good and, when the development speed is increased, the re-dispersibility is easy and the occurrence of stains by adhesion of the grains onto each part of the developing device is not observed.

Also, when the latex grains are fixed by heating, etc., a strong coating or layer having an excellent fixing property can be formed.

Furthermore, the liquid developer according to the present invention shows excellent dispersion stability, re-dispersibility, and fixing property when the liquid developer is used in a quickened development-fix step with a prolonged interval period of the maintenance or when a large size master plate is developed. Also, the liquid developer according to the present invention provides a master plate for offset printing having an excellent printing durability.

In particular, JP-A-62-166362, JP-A-63-66567, JP-A-60-185963 and JP-A-61-63855 disclose non-aqueous dispersed resins (latex grains) produced by polymeriza-

tion-granulation of a monomer which is insolubilized by polymerization, together with a monomer containing at least two ester bonds, etc. in the molecule which is copolymerizable with the above monomer or a monomer containing a long chain alkyl moiety, in the presence of a dispersion-stabilizing resin composed of a random copolymer which is soluble in a non-aqueous solvent and which contains copolymerizable components having polymerizable double bonds at the site apart from the polymer main chain by the total number of more than 8 atoms. These resin grains provide markedly improved dispersibility of resin grains and the printing durability as compared with conventional resin grains. However, they still have a problem in the redispersibility of resin grains when the liquid developer containing such resin grains is used in a plate-making machine for processing large size master plates for offset printing (e.g., ELP-560, ELP-820, etc. made by Fuji Photo Film Co., Ltd.) or when the liquid developer is used for plate-making at a high speed, thereby producing stains of plate-making machine (in particular, stains of developing device), causing aggregation and sedimentation of grains, or reducing the printing durability due to insufficient strength in the image areas. On the other hand, the liquid developer containing the dispersed resin according to the present invention has substantially no problems under the above-described severe conditions.

As described above, the high dispersibility of the latex grains of the present invention is fully dependent on the soluble graft type copolymer used in combination with the monomer (A) to be insolubilized, or the monomer (A) and the monomer (C) or (D).

That is, the characteristic feature of the present invention resides in that the dispersion-stabilizing resin is a graft type copolymer composed of an A block comprising polymer components containing a long chain aliphatic group having a high affinity for the non-aqueous solvent used, and a B block comprising polymer components having a low affinity for the non-aqueous solvent and a high affinity for the monomer (A) to be insolubilized.

Due to the above properties of the AB block copolymer used in the present invention, it is considered that the B block portion is well adsorbed onto the dispersed resin by physical and chemical mutual action during the polymerization-granulation, and the A block having a high affinity for the non-aqueous dispersion solvent is well solvated with the solvent and well produces steric repulsive effects (i.e., adsorbed in the tail form) thereby achieving the effect of the present invention.

On the other hand, in the conventional random copolymer composed of the polymerizable components used as the A block and the polymerizable components used as the B block, since the component as an adsorbing portion is randomly bonded in a high molecular weight chain composed of the components to be solvated, adsorption onto the dispersed resin grains is not sufficient and moreover the adsorption occurs in a loop form, the steric repulsive effect is decreased whereby stable dispersion cannot be obtained.

Further, it is considered that the high printing durability of the offset master plate resulting from less deterioration of the toner image during printing can be achieved by the formation of a uniform and stiff film, since the monomer (A) to be insolubilized and, optionally, the monomer (C) or (D), and the dispersed polymer adsorbed thereon have a good mutual solubility

and are sufficiently solubilized under mild fixing condition to form a uniform and stiff film.

The liquid developer of the present invention may contain, if desired, a colorant.

There is no specific restriction on the colorant being used, and any conventional pigments or dyes can be used as the colorant in the present invention.

In coloring the dispersion resin itself, for example, a method for coloring the dispersion resin by physically dispersing a pigment or dye in the dispersion resin can be used, and various pigments and dyes can be used for this purpose, for example, a magnetic iron oxide powder, a lead iodide powder, carbon black, nigrone, Alkali Blue, Hansa Yellow, quinacridone red, phthalocyanine blue, etc.

As another method for coloring the dispersion resin grains, the dispersion resin may be dyed with a desired dye, for example, as disclosed in JP-A-57-48738. As still another method, a dye may be chemically bonded to the dispersion resin as disclosed, for example, in JP-A-53-54029 or a previously dye-containing monomer is used in the polymerization granulation to provide a dye-containing dispersion resin as disclosed, for example, in JP-B-44-22955. (The term "JP-B" as used herein means an "examined Japanese patent publication".)

Various additives may be added to the liquid developer of the present invention for enhancing the charging characteristics or improving the image characteristics and they are practically described in Yuji Harasaki, *Electrophotography*, Vol. 16, No. 2, page 44.

Specific examples of these additives include metal salts of 2-ethylhexylsulfosuccinic acid, metal salts of naphthenic acid, metal salts of higher fatty acids, lecithin, poly(vinylpyrrolidone), and copolymers containing a semi-maleic acid amide component.

The amounts of the main constituting components of the liquid developer of the present invention are further described below.

The amount of the toner grains consisting essentially of the dispersion resin and, if desired, a colorant is preferably from about 0.5 to 50 parts by weight per 1,000 parts by weight of the liquid carrier. If the amount thereof is less than about 0.5 part by weight, the image density formed is insufficient and, if the amount exceeds about 50 parts by weight, non-image portions tend to be fogged. Further, the above-described liquid carrier-soluble resin for enhancing the dispersion stability may also be used, if desired, in an amount of from about 0.5 by weight to about 100 parts by weight per 1,000 parts by weight of the liquid carrier. Also, the charge-controlling agent as described above can be used preferably in an amount of from 0.001 part by weight to 1.0 part by weight per 1,000 parts by weight of the liquid carrier.

Furthermore, if desired, various additives may be added to the liquid developer, and the total amount of these additives is restricted by the electric resistance of the liquid developer. That is, if the electric resistance of the liquid developer in a state of excluding the toner grains therefrom becomes lower than  $10^9 \Omega\text{cm}$ , continuous tone images having good image quality are reluctant to obtain and, hence, it is necessary to control the amounts of additives in the above-described range of not lowering the electric resistance below  $10^9 \Omega\text{cm}$ .

The following examples are intended to illustrate the embodiments of the present invention in greater detail but not to limit the scope of the present invention in any way.

### SYNTHESIS EXAMPLE 1 OF MACROMONOMER (M): M-1

A mixed solution of 30 g of triphenylmethyl methacrylate and 100 g of toluene was sufficiently degassed under nitrogen gas stream and cooled to  $-20^\circ\text{C}$ . Then, 2 g of 1,1-diphenylbutyl lithium was added to the mixture, and the reaction was conducted for 10 hours. Separately, a mixed solution of 70 g of ethyl methacrylate and 100 g of toluene was sufficiently degassed under nitrogen gas stream, and the resulting mixed solution was added to the above described mixture, and then reaction was further conducted for 10 hours. The resulting mixture was adjusted to  $0^\circ\text{C}$ , and carbon dioxide gas was passed through the mixture in a flow rate of 60 ml/min for 30 minutes, then the polymerization reaction was terminated.

The temperature of the reaction solution obtained was raised to  $25^\circ\text{C}$ . under stirring, 6 g of 2-hydroxyethyl methacrylate was added thereto, then a mixed solution of 5 g of dicyclohexylcarbodiimide, 0.2 g of 4-N,N-dimethylaminopyridine and 10 g of methylene chloride was added dropwise thereto over a period of 30 minutes, and the mixture was stirred for 3 hours.

After removing the precipitated insoluble substances from the reaction mixture by filtration, 10 ml of an ethanol solution of 30% by weight hydrogen chloride was added to the filtrate, and the mixture was stirred for one hour. Then, the solvent of the reaction mixture was distilled off under reduced pressure until the whole volume was reduced to a half, and the mixture was reprecipitated from one liter of petroleum ether.

The precipitates thus formed were collected and dried under reduced pressure to obtain 56 g of Macromonomer (M-1) shown below having a weight average molecular weight of  $6.5 \times 10^3$ .



### SYNTHESIS EXAMPLE 2 OF MACROMONOMER (M): M-2

A mixed solution of 5 g of benzyl methacrylate, 0.5 g of (tetraphenyl porphinate) aluminum methyl, and 60 g of methylene chloride was raised to a temperature of  $30^\circ\text{C}$ . under nitrogen gas stream. The mixture was irradiated with light from a xenon lamp of 300 W at a distance of 25 cm through a glass filter, and the reaction was conducted for 12 hours. To the mixture was further added 45 g of butyl methacrylate, after similarly light-irradiating for 8 hours, 4 g of 4-bromomethylstyrene was added to the reaction mixture followed by stirring for 30 minutes, then the reaction was terminated. Then, Pd-C was added to the reaction mixture, and a catalytic reduction reaction was conducted for one hour at  $25^\circ\text{C}$ .

After removing insoluble substances from the reaction mixture by filtration, the reaction mixture was reprecipitated from 500 ml of petroleum ether, and the precipitates thus formed were collected and dried to obtain 33 g of Macromonomer (M-2) shown below having a weight average molecular weight of  $7 \times 10^3$ .



SYNTHESIS EXAMPLE 3 OF  
MACROMONOMER (M): M-3

A mixed solution of 20 g of 4-vinylphenoxytrimethylsilane and 100 g of toluene was sufficiently degassed under nitrogen gas stream and cooled to 0° C. Then, 2 g of 1,1-diphenyl-3-methylpentyl lithium was added to the mixture, followed by stirring for 6 hours. Separately, a mixed solution of 80 g of dodecyl methacrylate and 100 g of toluene was sufficiently degassed under nitrogen gas stream, and the resulting mixed solution was added to the above described mixture, and then reaction was further conducted for 8 hours. After introducing ethylene oxide in a flow rate of 30 ml/min into the reaction mixture for 30 minutes with thoroughly stirring, the mixture was cooled to a temperature of 15° C., and 10 g of methacrylic acid chloride was added dropwise thereto over a period of 30 minutes, followed by stirring for 3 hours.

Then, to the reaction mixture was added 10 ml of an ethanol solution of 30% by weight hydrogen chloride and, after stirring the mixture for one hour at 25° C., the mixture was reprecipitated from one liter of petroleum ether. The precipitates thus formed were collected, washed twice with 300 ml of diethyl ether and dried to obtain 55 g of Macromonomer (M-3) shown below having a weight average molecular weight of  $7.8 \times 10^3$ .



SYNTHESIS OF MACROMONOMER (M): M-4

A mixed solution of 40 g of triphenylmethyl acrylate and 100 g of toluene was sufficiently degassed under nitrogen gas stream and cooled to -20° C. Then, 0.2 g of sec-butyl lithium was added to the mixture, and the reaction was conducted for 10 hours. Separately, a mixed solution of 60 g of octadecylvinyl ether and 100 g of toluene was sufficiently degassed under nitrogen gas stream, and the resulting mixed solution was added to the above described mixture, and then reaction was

(M-2)

further conducted for 12 hours. The reaction mixture was adjusted to 0° C., 4 g of benzyl bromide was added thereto, and the reaction was conducted for one hour, followed by reacting at 25° C. for 2 hours.

Then, to the reaction mixture was added 10 g of an ethanol solution of 30% by weight hydrogen chloride, followed by stirring for 2 hours. After removing the insoluble substances from the reaction mixture by filtration, the mixture was reprecipitated from one liter of n-hexane. The precipitates thus formed were collected and dried under reduced pressure to obtain 58 g of Macromonomer (M-4) shown below having a weight average molecular weight of  $4.5 \times 10^3$ .



SYNTHESIS EXAMPLE 5 OF  
MACROMONOMER (M): M-5

A mixed solution of 80 g of octadecyl methacrylate and 4.8 g of benzyl N-hydroxyethyl-N-ethyldithiocarbamate was placed in a vessel under nitrogen gas stream followed by closing the vessel and heated to 60° C. The mixture was irradiated with light from a high-pressure mercury lamp for 400 W at a distance of 10 cm through a glass filter for 10 hours to conduct a photopolymerization.

Then, 30 g of acrylic acid and 180 g of methyl ethyl ketone were added to the mixture and, after replacing the gas in the vessel with nitrogen, the mixture was light-irradiated again for 10 hours.

To the reaction mixture was added dropwise 6 g of 2-isocyanatoethyl methacrylate at 30° C. over a period of one hour, and the mixture was stirred for 2 hours. The resulting reaction mixture was reprecipitated from 1.5 liters of hexane and the precipitates thus formed were collected and dried to obtain 68 g of Macromonomer (M-5) shown below having a weight average molecular weight of  $6.0 \times 10^3$ .



PRODUCTION EXAMPLE 1 OF  
DISPERSION-STABILIZING RESIN: P-1

A mixed solution of 80 g of octadecyl methacrylate, 20 g of Macromonomer M-1 and 150 g of toluene was warmed to a temperature of 75° C. under nitrogen gas stream. Then, 6 g of 2,2-azobis(isobutyronitrile) (abbreviated as A.I.B.N.) was added to the mixture, and the reaction was conducted for 4 hours. Then the reaction was further conducted for 6 hours while adding 2 g portion of A.I.B.N. at an interval of 3 hours. The resulting copolymer had a weight average molecular weight of  $5 \times 10^4$ .



PRODUCTION EXAMPLES 2 TO 12 OF  
DISPERSION-STABILIZING RESIN: P-2 to P-12

The polymers shown in Table 1 below were prepared by the polymerization method in the same manner as described in Production Example 1 of Dispersion-Stabilizing Resin. Each of the resulting polymers had a weight average molecular weight of from  $3 \times 10^4$  to  $6 \times 10^4$ .

PRODUCTION EXAMPLES 13 TO 35 OF  
DISPERSION-STABILIZING RESIN: P-13 TO P-35

The copolymers shown in Table 2 below were prepared under the same polymerization conditions as in Production Example 1 of Dispersion-Stabilizing Resin, except for using other macromonomers (M) in place of Macromonomer M-1 used in Production Example 1. Each of the resulting copolymers had a weight average molecular weight of from  $3 \times 10^4$  to  $7 \times 10^4$ .

TABLE 1

| Production Example | Resin P | $r_1$          | $-R$                          | $-Y-$                                                                                                           | $x/y$ |
|--------------------|---------|----------------|-------------------------------|-----------------------------------------------------------------------------------------------------------------|-------|
| 2                  | P-2     | $-\text{CH}_3$ | $-\text{C}_{18}\text{H}_{37}$ | $\begin{array}{c} \text{CH}_2-\text{CH}- \\   \\ \text{COOC}_{12}\text{H}_{25} \end{array}$                     | 50/30 |
| 3                  | P-3     | $-\text{CH}_3$ | $-\text{C}_{12}\text{H}_{25}$ | —                                                                                                               | 80/0  |
| 4                  | P-4     | $-\text{CH}_3$ | $-\text{C}_{13}\text{H}_{27}$ | $\begin{array}{c} \text{CH}_2-\text{CH}- \\   \\ \text{COOC}_{18}\text{H}_{37} \end{array}$                     | 40/40 |
| 5                  | P-5     | $-\text{H}$    | $-\text{C}_{18}\text{H}_{37}$ | —                                                                                                               | 80/0  |
| 6                  | P-6     | $-\text{H}$    | $-\text{C}_{12}\text{H}_{25}$ | $\begin{array}{c} \text{CH}_3 \\   \\ -\text{CH}_2-\text{C}- \\   \\ \text{COOC}_{12}\text{H}_{25} \end{array}$ | 60/20 |
| 7                  | P-7     | $-\text{CH}_3$ | $-\text{C}_{14}\text{H}_{29}$ | —                                                                                                               | 80/0  |
| 8                  | P-8     | $-\text{CH}_3$ | $-\text{C}_{16}\text{H}_{33}$ | —                                                                                                               | 80/0  |
| 9                  | P-9     | $-\text{CH}_3$ | $-\text{C}_{18}\text{H}_{37}$ | $\begin{array}{c} \text{CH}_3 \\   \\ -\text{CH}_2-\text{C}- \\   \\ \text{COOC}_{12}\text{H}_{25} \end{array}$ | 30/50 |
| 10                 | P-10    | $-\text{CH}_3$ | $-\text{C}_{12}\text{H}_{25}$ | $\begin{array}{c} \text{CH}_2-\text{CH}- \\   \\ \text{COOC}_{18}\text{H}_{37} \end{array}$                     | 50/30 |
| 11                 | P-11    | $-\text{CH}_3$ | $-\text{C}_{18}\text{H}_{37}$ | $\begin{array}{c} \text{CH}_3 \\   \\ -\text{CH}_2-\text{C}- \\   \\ \text{COOC}_4\text{H}_9 \end{array}$       | 70/10 |
| 12                 | P-12    | $-\text{H}$    | $-\text{C}_{12}\text{H}_{25}$ | $\begin{array}{c} \text{CH}_2-\text{CH}- \\   \\ \text{COOC}_{18}\text{H}_{37} \end{array}$                     | 40/40 |

TABLE 2

| Production Example | Resin P | X                                           | $\alpha_1/\alpha_2$ | -R                                 | $\chi/y$ (weight ratio)                             |                                                      |
|--------------------|---------|---------------------------------------------|---------------------|------------------------------------|-----------------------------------------------------|------------------------------------------------------|
|                    |         |                                             |                     |                                    | -H/-CH <sub>3</sub>                                 | -COOCH <sub>3</sub>                                  |
| 13                 | P-13    | -COO(CH <sub>2</sub> ) <sub>2</sub> OOC-    |                     | -H/-CH <sub>3</sub>                | -COOCH <sub>3</sub>                                 | -CH <sub>2</sub> -CH-                                |
|                    |         |                                             |                     |                                    |                                                     | COOH                                                 |
| 14                 | P-14    | -COOCH <sub>2</sub> CH(CH <sub>2</sub> OOC- |                     | -CH <sub>3</sub> /-CH <sub>3</sub> | -COOCH <sub>2</sub> C <sub>6</sub> H <sub>5</sub>   | -CH <sub>2</sub> -CH-                                |
|                    |         | OH                                          |                     |                                    |                                                     | COOH                                                 |
| 15                 | P-15    |                                             |                     | -H/-CH <sub>3</sub>                | -COOC <sub>10</sub> H <sub>21</sub>                 |                                                      |
|                    |         |                                             |                     |                                    |                                                     | COOH                                                 |
| 16                 | P-16    |                                             |                     | -CH <sub>3</sub> /-CH <sub>3</sub> | -COOC <sub>2</sub> H <sub>5</sub>                   |                                                      |
|                    |         |                                             |                     |                                    |                                                     | COOH                                                 |
| 17                 | P-17    | -COOCH <sub>2</sub> CH <sub>2</sub> -       |                     | -CH <sub>3</sub> /-CH <sub>3</sub> | -C <sub>6</sub> H <sub>5</sub>                      |                                                      |
|                    |         |                                             |                     |                                    |                                                     | OH                                                   |
| 18                 | P-18    | -COOCH <sub>2</sub> CH(CH <sub>2</sub> OOC- |                     | -CH <sub>3</sub> /-CH <sub>3</sub> | -COOCH <sub>2</sub> C <sub>12</sub> H <sub>25</sub> |                                                      |
|                    |         | OH                                          |                     |                                    |                                                     | COO(CH <sub>2</sub> ) <sub>3</sub> SO <sub>3</sub> H |

TABLE 2-continued

| Production Example | Resin P | X | $\frac{a_1}{a_2}$ | $-R$            | $-R'$           | $\frac{x}{y}$<br>(weight ratio) |       |
|--------------------|---------|---|-------------------|-----------------|-----------------|---------------------------------|-------|
| 19                 | P-19    |   |                   | $-H/-CH_3$      | $-COOCCH_3H_2$  |                                 | 80/20 |
| 20                 | P-20    |   |                   | $-CH_3/-CH_3$   | $-COOC_6H_5H_2$ |                                 | 65/35 |
| 21                 | P-21    | " |                   | $-CH_3/-H$      | $-COOC_6H_5H_2$ |                                 | 70/30 |
| 22                 | P-22    |   |                   | $-CH_3/-CH_3$   | $-COOCH_3$      |                                 | 75/25 |
| 23                 | P-23    |   |                   | $-COOCH_2CH_2-$ | $-C_6H_5-$      |                                 | 90/10 |

TABLE 2-continued

| Production<br>Ex-<br>ample | Resin P | X                                                                                    | a <sub>1</sub> /a <sub>2</sub> | —R                                 | —Z—                                               | x/y<br>(weight<br>ratio) |
|----------------------------|---------|--------------------------------------------------------------------------------------|--------------------------------|------------------------------------|---------------------------------------------------|--------------------------|
| 24                         | P-24    |    |                                | —CH <sub>3</sub> /—CH <sub>3</sub> | —COOCH <sub>2</sub> C <sub>6</sub> H <sub>5</sub> | 70/30                    |
| 25                         | P-25    |    |                                | —H/—CH <sub>3</sub>                | —COOC <sub>4</sub> H <sub>9</sub>                 | 80/20                    |
| 26                         | P-26    |    |                                | —CH <sub>3</sub> /—CH <sub>3</sub> | —COOC <sub>12</sub> H <sub>25</sub>               | 60/40                    |
| 27                         | P-27    |  |                                | —CH <sub>3</sub> /—CH <sub>3</sub> | —COOC <sub>8</sub> H <sub>17</sub>                | 70/30                    |
| 28                         | P-28    |  |                                | —H/—H                              | —COOC <sub>12</sub> H <sub>25</sub>               | 60/40                    |
| 29                         | P-29    |  |                                | —H/—CH <sub>3</sub>                | —COOC <sub>14</sub> H <sub>29</sub>               | 85/15                    |

TABLE 2-continued

| Production Example | Resin P | X                                                                                   | a <sub>1</sub> /a <sub>2</sub> | -R                                       | -Z-                                 | x/y (weight ratio)                  |
|--------------------|---------|-------------------------------------------------------------------------------------|--------------------------------|------------------------------------------|-------------------------------------|-------------------------------------|
| 30                 | P-30    |    |                                | -H/-CH <sub>3</sub>                      | -COOC <sub>18</sub> H <sub>37</sub> | 80/20                               |
| 31                 | P-31    |    |                                | -COO-                                    | -CH <sub>3</sub> /-H                | -COOC <sub>12</sub> H <sub>25</sub> |
| 32                 | P-32    |    |                                | -COO(CH <sub>2</sub> ) <sub>2</sub> OOC- | -CH <sub>3</sub> /-CH <sub>3</sub>  | -COOC <sub>4</sub> H <sub>9</sub>   |
| 33                 | P-33    | "                                                                                   | "                              | -H/-CH <sub>3</sub>                      | -COOC <sub>18</sub> H <sub>37</sub> | 75/25                               |
| 34                 | P-34    | "                                                                                   | "                              | -H/-CH <sub>3</sub>                      | -COOC <sub>8</sub> H <sub>17</sub>  | 70/30                               |
| 35                 | P-35    |  |                                | -CH <sub>3</sub> /-CH <sub>3</sub>       | -COOC <sub>12</sub> H <sub>25</sub> | 90/10                               |

**PRODUCTION EXAMPLE 1 OF LATEX  
GRAINS: D-1**

A mixed solution of 10 g of the dispersion-stabilizing resin P-1, 100 g of vinyl acetate, and 380 g of Isopar H was heated to 75° C. with stirring under nitrogen gas stream. Then, after adding thereto 1.0 g of 2,2'-azobisisobutyronitrile (abbreviated as A.I.V.N.), as a polymerization initiator, the reaction was carried out for 2 hours, and, after further adding 0.6 g of A.I.V.N., the reaction was conducted for 2 hours.

20 minutes after the addition of the polymerization initiator, the reaction mixture became white-turbid, and the reaction temperature raised to 88° C. Then, the temperature of the reaction mixture was raised to 100° C. and stirred for 2 hours to distil off unreacted vinyl acetate. After cooling, the reaction mixture was passed through a 200 mesh nylon cloth so as to remove coarse grains to obtain the desired latex having a mean grain size of 0.22 µm with a polymerization ratio of 86% as a white dispersion.

**PRODUCTION EXAMPLES 2 TO 18 OF LATEX  
GRAINS: D-2 to D-18**

By following the same procedure as Production Example 1 of latex grains except that each of the dispersion-stabilizing resins described in Table 3 below was used in place of the dispersion-stabilizing resin P-1, each of the latex grains D-2 to D-18 was produced.

TABLE 3

| Production Example of Latex Grains | Latex Grains | Dispersion-Stabilizing Resin and Amount | Latex Grain              |                      |
|------------------------------------|--------------|-----------------------------------------|--------------------------|----------------------|
|                                    |              |                                         | Polymerization Ratio (%) | Mean Grain Size (µm) |
| 2                                  | D-2          | P-2                                     | 12 g                     | 83                   |
| 3                                  | D-3          | P-3                                     | 11 g                     | 85                   |
| 4                                  | D-4          | P-4                                     | 13 g                     | 86                   |
| 5                                  | D-5          | P-5                                     | 12 g                     | 85                   |
| 6                                  | D-6          | P-11                                    | 14 g                     | 86                   |
| 7                                  | D-7          | P-12                                    | 11 g                     | 88                   |
| 8                                  | D-8          | P-13                                    | 13 g                     | 86                   |
| 9                                  | D-9          | P-15                                    | 12 g                     | 85                   |
| 10                                 | D-10         | P-18                                    | 14 g                     | 86                   |
| 11                                 | D-11         | P-19                                    | 12 g                     | 87                   |
| 12                                 | D-12         | P-24                                    | 14 g                     | 85                   |
| 13                                 | D-13         | P-25                                    | 12 g                     | 86                   |
| 14                                 | D-14         | P-26                                    | 12 g                     | 87                   |
| 15                                 | D-15         | P-28                                    | 12 g                     | 86                   |
| 16                                 | D-16         | P-29                                    | 11 g                     | 87                   |
| 17                                 | D-17         | P-32                                    | 14 g                     | 85                   |
| 18                                 | D-18         | P-33                                    | 12 g                     | 86                   |

**PRODUCTION EXAMPLE 19 OF LATEX  
GRAINS: D-19**

A mixed solution of 85 g of vinyl acetate, 15 g of N-vinylpyrrolidone, 12 g of the dispersion-stabilizing resin P-31, and 380 g of n-decane was heated to 75° C. with stirring under nitrogen gas stream. Then, after adding 1.7 g of 2,2'-azobisisobutyronitrile (abbreviated as A.I.B.N.) to the reaction mixture, the reaction was carried out for 4 hours and, after further adding thereto 0.5 g of A.I.B.N., the reaction was carried out for 2 hours. After cooling, the reaction mixture obtained was passed through a 200 mesh nylon cloth to obtain the desired latex grains having a mean grain size of 0.25 µm as a white dispersion.

**PRODUCTION EXAMPLE 20 OF LATEX  
GRAINS: D-20**

A mixed solution of 20 g of the dispersion-stabilizing resin P-13 and 470 g of n-dodecane was heated to 60° C. with stirring under nitrogen gas stream. Then, a mixed solution of 100 g of methyl methacrylate, 1.0 g of n-dodecylmercaptan and 0.8 g of A.I.V.N. was added dropwise to the reaction mixture over a period of 2 hours, and the resulting mixture was reacted for 2 hours as it was. 0.3 g of A.I.V.N. was further added thereto, the mixture was reacted for 2 hours. After cooling, the reaction mixture obtained was passed through a 200 mesh nylon cloth to obtain the desired latex grains having a mean grain size of 0.28 µm as a white dispersion.

**PRODUCTION EXAMPLE 21 OF LATEX  
GRAINS: D-21**

A mixed solution of 14 g of the dispersion-stabilizing resin P-21, 100 g of vinyl acetate, 5 g of crotonic acid and 468 g of Isopar E was heated to 70° C. with stirring under nitrogen gas stream and, after adding 0.8 g of A.I.V.N. to the reaction mixture, the reaction was carried out for 6 hours. The temperature was elevated to 100° C., and the mixture was stirred at that temperature for 1 hour to distil off remaining vinyl acetate. After cooling, the reaction mixture was passed through a 200 mesh nylon cloth in order to remove coarse grains to obtain latex grains having a mean grain size of 0.24 µm with a polymerization ratio of 85% as a white dispersion.

**PRODUCTION EXAMPLE 22 OF LATEX  
GRAINS: D-22**

A mixed solution of 14 g of the dispersion-stabilizing resin P-25, 100 g of vinyl acetate, 6.0 g of 4-pentenoic acid and 380 g of Isopar G was heated to 75° C. with stirring under nitrogen gas stream. Then, after adding 0.7 g of A.B.V.N. to the reaction mixture, the reaction was carried out for 4 hours and, after further adding thereto 0.5 g of A.B.V.N., the reaction was carried out for 2 hours. After cooling, the reaction mixture was passed through a 200 mesh nylon cloth so as to remove coarse grains to obtain latex grains having a mean grain size of 0.23 µm as a white dispersion.

**PRODUCTION EXAMPLE 23 OF LATEX  
GRAINS: D-23**

A mixed solution of 100 g of styrene, 20 g of the dispersion-stabilizing resin P-27, and 380 g of Isopar H was heated to 60° C. with stirring under nitrogen gas stream and, after adding 0.6 g of A.I.V.N. to the reaction mixture, the reaction was carried out for 4 hours. Then, after further adding thereto 0.3 g of A.I.V.N., the reaction was carried out for 3 hours. After cooling, the reaction mixture was passed through a 200 mesh nylon cloth so as to remove coarse grains to obtain the desired latex grains having a mean grain size of 0.23 µm as a white dispersion.

**PRODUCTION EXAMPLE 24 OF LATEX  
GRAINS: D-24**

By following the same procedure as Production Example 23 of latex grains D-23 except that a mixed solution of 40 g of styrene, 60 g of vinyltoluene, 20 g of the dispersion-stabilizing resin P-17 and 380 g of Isopar H was used in place of the mixture used in Example 23, latex grains having a mean grain size of 0.24 µm were

obtained with a polymerization ratio of 80% as a white dispersion.

#### PRODUCTION EXAMPLE 25 OF LATEX GRAINS: COMPARATIVE EXAMPLE A

By following the same procedure as Production Example 1 of latex grains D-1 except that a mixed solution of 20 g of poly(octadecyl methacrylate), 100 g of vinyl acetate, 1.0 g of octadecyl methacrylate and 385 g of Isopar H was used in place of the mixture used in Production Example 1, latex grains having a mean grain size of 0.20  $\mu\text{m}$  were obtained with a polymerization ratio of 85% as a white dispersion. (Latex grains disclosed in JP-A-60-179751).

#### PRODUCTION EXAMPLE 26 OF LATEX GRAINS: COMPARATIVE EXAMPLE B

By following the same procedure as Production Example 1 of latex grains D-1 except that a mixed solution of 10 g of a dispersion-stabilizing resin R-1 having the formula shown below, 100 g of vinyl acetate, 1 g of Monomer (I) having the formula shown below, and 385 g of Isopar H was used in place of the mixture used in Production Example 1, latex grains having a mean grain size of 0.24  $\mu\text{m}$  were obtained with the polymerization ratio of 86% as a white dispersion. (Latex grains disclosed in JP-A-63-66567).

Monomer (I)



Dispersion-Stabilizing Resin: R-1



#### PRODUCTION EXAMPLE 27 OF LATEX GRAINS: D-27

A mixed solution of 14 g of the dispersion-stabilizing resin P-1, 100 g of vinyl acetate, 1.5 g of Compound III-19 of Monomer (C) and 384 g of Isopar H was heated to 70° C. with stirring under nitrogen gas stream. Then, after adding thereto 0.8 g of 2,2'-azobisis(isovaleronitrile) (A.I.V.N.) as a polymerization initiator, the reaction was carried out for 6 hours. 20 minutes after the addition of the polymerization initiator, the reaction mixture became whiteturbid, and the reaction temperature raised to 88° C. Then, the temperature of the reaction mixture was raised to 100° C. and stirred for 2 hours to distill off unreacted vinyl acetate. After cooling, the reaction mixture was passed through a 200 mesh nylon cloth to obtain the desired latex having a mean grain size of 0.24  $\mu\text{m}$  with a polymerization ratio of 86% as a white dispersion.

#### PRODUCTION EXAMPLES 28 TO 44 OF LATEX GRAINS: D-28 TO D-44

By following the same procedure as Production Example 27 of latex grains except that each of the dispersion-stabilizing resins described in Table 4 below was used in place of the dispersion-stabilizing resin P-1, each of the latex grains D-28 to D-44 was produced.

TABLE 4

| Production Example of Latex Grains | Latex Grains | Dispersion-Stabilizing Resin and Amount | Latex Grain              |                                   |
|------------------------------------|--------------|-----------------------------------------|--------------------------|-----------------------------------|
|                                    |              |                                         | Polymerization Ratio (%) | Mean Grain Size ( $\mu\text{m}$ ) |
| 5                                  | 28           | D-28 P-2                                | 12 g 83                  | 0.23                              |
|                                    | 29           | D-29 P-3                                | 11 g 85                  | 0.25                              |
|                                    | 30           | D-30 P-4                                | 13 g 86                  | 0.22                              |
|                                    | 31           | D-31 P-5                                | 12 g 85                  | 0.20                              |
| 10                                 | 32           | D-32 P-11                               | 14 g 86                  | 0.24                              |
|                                    | 33           | D-33 P-12                               | 11 g 88                  | 0.20                              |
|                                    | 34           | D-34 P-13                               | 13 g 86                  | 0.22                              |
|                                    | 35           | D-35 P-15                               | 12 g 85                  | 0.24                              |
|                                    | 36           | D-36 P-18                               | 14 g 86                  | 0.20                              |
| 15                                 | 37           | D-37 P-19                               | 12 g 87                  | 0.19                              |
|                                    | 38           | D-38 P-24                               | 14 g 85                  | 0.21                              |
|                                    | 39           | D-39 P-25                               | 12 g 86                  | 0.22                              |
|                                    | 40           | D-40 P-26                               | 12 g 87                  | 0.23                              |
|                                    | 41           | D-41 P-28                               | 12 g 86                  | 0.22                              |
|                                    | 42           | D-42 P-29                               | 11 g 87                  | 0.23                              |
| 20                                 | 43           | D-43 P-32                               | 14 g 85                  | 0.25                              |
|                                    | 44           | D-44 P-33                               | 12 g 86                  | 0.22                              |

#### PRODUCTION EXAMPLES 45 TO 65 OF LATEX GRAINS: D-45 TO D-65

By following the same procedure as Production Example 27 of latex grains except that dispersion-stabilizing resin and the monomer (C) shown in Table 5 below were used in place of the dispersion-stabilizing resin P-1 and Compound III-19 as monomer (C), respectively, each of the latex grains D-45 to D-65 was produced. The polymerization ratios of the latex grains obtained were from 85 to 90%. Also, the mean grain size of the resulting latex grains was in the range of from 0.18 to 0.25  $\mu\text{m}$ , and the latex had excellent mono-dispersibility.

TABLE 5

| Production Example of Latex Grains | Latex Grains | Dispersion-Stabilizing Resin | Monomer (C) |
|------------------------------------|--------------|------------------------------|-------------|
| 40                                 | 45           | D-45 P-1                     | III-1       |
|                                    | 46           | D-46 "                       | III-2       |
|                                    | 47           | D-47 "                       | III-3       |
|                                    | 48           | D-48 "                       | III-8       |
|                                    | 49           | D-49 "                       | III-9       |
|                                    | 50           | D-50 "                       | III-10      |
|                                    | 51           | D-51 "                       | III-11      |
|                                    | 52           | D-52 "                       | III-14      |
|                                    | 53           | D-53 "                       | III-18      |
|                                    | 54           | D-54 P-2                     | III-10      |
|                                    | 55           | D-55 P-3                     | III-19      |
|                                    | 56           | D-56 P-5                     | III-20      |
| 50                                 | 57           | D-57 P-5                     | III-21      |
|                                    | 58           | D-58 P-7                     | III-22      |
|                                    | 59           | D-59 P-7                     | III-23      |
|                                    | 60           | D-60 P-7                     | III-24      |
|                                    | 61           | D-61 P-8                     | III-15      |
|                                    | 62           | D-62 P-8                     | III-16      |
|                                    | 63           | D-63 P-8                     | III-26      |
|                                    | 64           | D-64 P-2                     | III-27      |
| 55                                 | 65           | D-65 P-3                     | III-29      |

#### PRODUCTION EXAMPLE 66 OF LATEX GRAINS: D-66

By following the same procedure as Production Example 27 of latex grains except that each of the dispersion-stabilizing resins described in Table 4 below was used in place of the dispersion-stabilizing resin P-1, each of the latex grains D-28 to D-44 was produced.

and, after further adding thereto 0.5 g of A.I.B.N., the reaction was carried out for 2 hours. The temperature of the reaction mixture was elevated to 110° C., and the reaction mixture was stirred for 2 hours to distil off the low-boiling solvent and remaining vinyl acetate. After cooling, the reaction mixture was passed through a 200 mesh nylon cloth to obtain the desired latex grains having a mean grain size of 0.18  $\mu\text{m}$  as a white dispersion.

**PRODUCTION EXAMPLE 67 OF LATEX GRAINS: D-67**

A mixed solution of 14 g of the dispersion-stabilizing resin P-31, 90 g of vinyl acetate, 2.0 g of Compound III-23 as monomer (C), 10 g of N-vinylpyrrolidone, and 400 g of isododecane was heated to 65° C. with stirring under nitrogen gas stream and, after adding 1.5 g of A.I.B.N. to the reaction mixture, the reaction was carried out for 4 hours. After cooling, the reaction mixture was passed through a 200 mesh nylon cloth to obtain the desired latex grains having a mean grain size of 0.26  $\mu\text{m}$  as a white dispersion.

**PRODUCTION EXAMPLE 68 OF LATEX GRAINS: D-68**

A mixed solution of 16 g of the dispersion-stabilizing resin P-4, 94 g of vinyl acetate, 6 g of 4-pentenoic acid, 1.5 g of Compound III-19 as monomer (C), and 380 g of Isopar G was heated to 60° C. with stirring under nitrogen gas stream. Then, after adding 1.0 g of A.I.V.N. to the reaction mixture, the reaction was carried out for 2 hours and, after further adding thereto 0.5 g of A.I.V.N., the reaction was carried out for 2 hours. After cooling, the reaction mixture was passed through a 200 mesh nylon cloth to obtain the desired latex grains having a mean grain size of 0.24  $\mu\text{m}$  as a white dispersion.

**PRODUCTION EXAMPLE 69 OF LATEX GRAINS: D-69**

A mixed solution of 20 g of the dispersion-stabilizing resin P-32, 2 g of Compound III-17 as monomer (C), 1.2 g of n-dodecylmercaptan, 100 g of methyl methacrylate, and 688 g of Isopar H was heated to 65° C. with stirring under nitrogen gas stream and, after adding 1.2 g of A.I.V.N. to the reaction mixture, the reaction was carried out for 4 hours. After cooling, the reaction mixture was passed through a 200 mesh nylon cloth so as to remove coarse grains to obtain the desired latex grains having a mean grain size of 0.28  $\mu\text{m}$  as a white dispersion.

**PRODUCTION EXAMPLE 70 OF LATEX GRAINS: D-70**

A mixed solution of 18 g of the dispersion-stabilizing resin P-13, 100 g of vinyl acetate, 5 g of crotonic acid, 2 g of Compound III-29 as monomer (C) and 468 g of Isopar E was heated to 70° C. with stirring under nitrogen gas stream and, after adding 0.8 g of A.I.V.N. to the reaction mixture, the reaction was carried out for 6 hours. The temperature was elevated to 100° C., and the mixture was stirred for one hour to distil off the remaining vinyl acetate. After cooling, the reaction mixture was passed through a 200 mesh nylon cloth so as to remove coarse grains to obtain the desired latex grains having a mean grain size of 0.26  $\mu\text{m}$  with a polymerization ratio of 85% as a white dispersion.

**PRODUCTION EXAMPLE 71 OF LATEX GRAINS: D-71**

5 A mixed solution of 20 g of the dispersion-stabilizing resin P-17, 100 g of styrene, 4 g of Compound III-25 as monomer (C), and 380 g of Isopar H was heated to 50° C. with stirring under nitrogen gas stream and, after adding 1.0 g (as solid content) of a hexane solution of n-butyl lithium to the reaction mixture, the reaction was 10 carried out for 4 hours. After cooling, the reaction mixture was passed through a 200 mesh nylon cloth to obtain desired latex grains having a mean grain size of 0.27  $\mu\text{m}$  as a white dispersion.

**PRODUCTION EXAMPLE 72 OF LATEX GRAINS: D-72**

A mixed solution of 20 g of the dispersion-stabilizing resin P-33 and 680 g of n-dodecane was heated to 60° C. with stirring under nitrogen gas stream. Then, a mixed 20 solution of 100 g of methyl methacrylate, 1.0 g of n-dodecylmercaptan, 3 g of Compound III-1 as monomer (C) and 0.8 g of A.I.V.N. was added dropwise to the above solution over 2 hours. After reacting the mixture for 2 hours, 0.3 g of A.I.V.N. was further added thereto, 25 followed by reacting the mixture for 2 hours. After cooling, the reaction mixture was passed through a 200 mesh nylon cloth so as to remove coarse grains to obtain the desired latex grains having a mean grain size of 0.25  $\mu\text{m}$  as a white dispersion.

**PRODUCTION EXAMPLE 73 OF LATEX GRAINS: COMPARATIVE EXAMPLE C**

By following the same procedure as Production Example 27 of latex grains D-27 except that a mixed solution of 20 g of poly(octadecyl methacrylate), 100 g of vinyl acetate, 1.2 g of Monomer (I) having the formula shown below and 385 g of Isopar H was used in place of the mixture used in Production Example 27, latex grains having a mean grain size of 0.23  $\mu\text{m}$  were obtained with a polymerization ratio of 85% as a white dispersion. (Latex grains disclosed in JP-A-62-166362).

**PRODUCTION EXAMPLE 74 OF LATEX GRAINS: COMPARATIVE EXAMPLE D**

By following the same procedure as Production Example 27 of latex grains D-27 except that a mixed solution of 10 g of a dispersion-stabilizing resin R-1 having the formula shown below, 100 g of vinyl acetate, 1 g of Monomer (I) having the formula shown below, and 385 g of Isopar H was used in place of the mixture used in Production Example 27, latex grains having a mean grain size of 0.24  $\mu\text{m}$  were obtained with the polymerization ratio of 86% as a white dispersion. (Latex grains disclosed in JP-A-60-66567).

55 Monomer (I)



60 Dispersion-Stabilizing Resin: R-1



PRODUCTION EXAMPLE 75 OF LATEX  
GRAINS: D-75

A mixed solution of 15 g of the dispersion-stabilizing resin P-1, 100 g of vinyl acetate, 1.0 g of octadecyl methacrylate, and 384 g of Isopar H was heated to 70° C. with stirring under nitrogen gas stream and, after adding 0.8 g of A.I.V.N. to the reaction mixture, the reaction was carried out for 6 hours. Twenty minutes after the addition of the polymerization initiator, the reaction mixture became white-turbid, and the reaction temperature raised to 88° C. Then, after raising the temperature to 100° C., the reaction mixture was stirred for 2 hours to distil off unreacted vinyl acetate. After cooling, the reaction mixture was passed through a 200 mesh nylon cloth to obtain the desired latex grains having a mean grain size of 0.24  $\mu\text{m}$  with a polymerization ratio of 90% as a white dispersion.

PRODUCTION EXAMPLES 76 TO 92 OF LATEX  
GRAINS: D-76 TO D-92

By following the same procedure as Production Example 75 of Latex Grains except that each of the dispersion-stabilizing resins described in Table 6 below was used in place of the dispersion-stabilizing resin P-1, each of the Latex Grains D-76 to D-92 was obtained.

TABLE 6

| Production Example of Latex Grains | Latex Grains | Dispersion-Stabilizing Resin and Amount | Latex Grain              |                                   | Mean Grain Size ( $\mu\text{m}$ ) |
|------------------------------------|--------------|-----------------------------------------|--------------------------|-----------------------------------|-----------------------------------|
|                                    |              |                                         | Polymerization Ratio (%) | Mean Grain Size ( $\mu\text{m}$ ) |                                   |
| 76                                 | D-76         | P-2                                     | 12 g                     | 83                                | 0.23                              |
| 77                                 | D-77         | P-3                                     | 11 g                     | 85                                | 0.25                              |
| 78                                 | D-78         | P-4                                     | 13 g                     | 86                                | 0.22                              |
| 79                                 | D-79         | P-5                                     | 12 g                     | 85                                | 0.20                              |
| 80                                 | D-80         | P-11                                    | 14 g                     | 86                                | 0.24                              |
| 81                                 | D-81         | P-12                                    | 11 g                     | 88                                | 0.20                              |
| 82                                 | D-82         | P-13                                    | 13 g                     | 86                                | 0.22                              |
| 83                                 | D-83         | P-15                                    | 12 g                     | 85                                | 0.24                              |
| 84                                 | D-84         | P-18                                    | 14 g                     | 86                                | 0.20                              |
| 85                                 | D-85         | P-19                                    | 12 g                     | 87                                | 0.19                              |
| 86                                 | D-86         | P-24                                    | 14 g                     | 85                                | 0.21                              |
| 87                                 | D-87         | P-25                                    | 12 g                     | 86                                | 0.22                              |
| 88                                 | D-88         | P-26                                    | 12 g                     | 87                                | 0.23                              |
| 89                                 | D-89         | P-28                                    | 12 g                     | 86                                | 0.22                              |
| 90                                 | D-90         | P-29                                    | 11 g                     | 87                                | 0.23                              |
| 91                                 | D-91         | P-32                                    | 14 g                     | 85                                | 0.25                              |
| 92                                 | D-92         | P-33                                    | 12 g                     | 86                                | 0.22                              |

PRODUCTION EXAMPLES 93 TO 98 OF LATEX  
GRAINS: D-93 TO D-98

By following the same procedure as Production Example 75 of latex grains except that 0.8 g of each of the monomers shown in Table 7 was used in place of 1 g of octadecyl methacrylate used in Production Example 75, each of latex grains was produced.

TABLE 7

| Production Example of Latex Grains | Latex Grains | Monomer                 | Latex Grains             |                                   | Mean Grain Size ( $\mu\text{m}$ ) |
|------------------------------------|--------------|-------------------------|--------------------------|-----------------------------------|-----------------------------------|
|                                    |              |                         | Polymerization Ratio (%) | Mean Grain Size ( $\mu\text{m}$ ) |                                   |
| 93                                 | D-93         | Docosanyl Methacrylate  | 87                       | 0.23                              |                                   |
| 94                                 | D-94         | Hexadecyl Methacrylate  | 87                       | 0.24                              |                                   |
| 95                                 | D-95         | Tetradecyl Methacrylate | 88                       | 0.24                              |                                   |
| 96                                 | D-96         | Tridecyl Methacrylate   | 86                       | 0.24                              |                                   |
| 97                                 | D-97         | Dodecyl Methacrylate    | 86                       | 0.23                              |                                   |
| 98                                 | D-98         | Decyl Methacrylate      | 87                       | 0.26                              |                                   |

PRODUCTION EXAMPLE 99 OF LATEX  
GRAINS: D-99

A mixed solution of 10 g of the dispersion-stabilizing resin P-10, 4 g of poly(octadecyl methacrylate) 100 g of vinyl acetate, 0.8 g of dodecyl methacrylate, and 400 g of Isopar H was heated to 75° C. with stirring under nitrogen gas stream. Then, after adding 0.7 g of 2,2'-azobis(isobutyronitrile) (abbreviated as A.I.B.N.) to the reaction mixture, the reaction was carried out for 4 hours and, after further adding thereto 0.5 g of A.I.B.N., the reaction was carried out for 2 hours. After cooling, the reaction mixture was passed through a 200 mesh nylon cloth to obtain the desired latex grains having a mean grain size of 0.20  $\mu\text{m}$  as a white dispersion.

PRODUCTION EXAMPLE 100 OF LATEX  
GRAINS: D-100

A mixed solution of 14 g of the dispersion-stabilizing resin P-11, 90 g of vinyl acetate, 10 g of N-vinylpyrrolidone, 1.5 g of octadecyl methacrylate, and 400 g of isododecane was heated to 65° C. with stirring under nitrogen gas stream and, after adding 1.5 g of A.I.B.N. to the reaction mixture, the reaction was carried out for 4 hours. After cooling, the reaction mixture was passed through a 200 mesh nylon cloth to obtain the desired latex grains having a mean grain size of 0.25  $\mu\text{m}$  as a white dispersion.

PRODUCTION EXAMPLE 101 OF LATEX  
GRAINS: D-101

A mixed solution of 16 g of the dispersion-stabilizing resin P-4, 94 g of vinyl acetate, 6 g of crotonic acid, 2 g of hexadecyl methacrylate, and 378 g of Isopar G was heated to 60° C. with stirring under nitrogen gas stream. After adding 1.0 g of A.I.V.N. to the reaction mixture, the reaction was carried out for 2 hours and, after further adding thereto 0.5 g of A.I.V.N., the reaction was carried out for 2 hours. After cooling, the reaction mixture was passed through a 200 mesh nylon cloth to obtain the desired latex grains having a mean grain size of 0.24  $\mu\text{m}$  as a white dispersion.

PRODUCTION EXAMPLE 102 OF LATEX  
GRAINS: D-102

A mixed solution of 25 g of the dispersion-stabilizing resin P-7, 100 g of methyl methacrylate, 2 g of dodecyl acrylate, 0.8 g of n-dodecylmercaptan, and 688 g of Isopar H was heated to 60° C. with stirring under nitrogen gas stream and, after adding 0.7 g of A.I.V.N. to the reaction mixture, the reaction was carried out for 4 hours. After cooling, the reaction mixture was passed through a 200 mesh nylon cloth to obtain the desired latex grains having a mean grain size of 0.25  $\mu\text{m}$  as a white dispersion.

PRODUCTION EXAMPLE 103 OF LATEX  
GRAINS: D-103

A mixed solution of 20 g of the dispersion-stabilizing resin P-17, 100 g of styrene, 2 g of octadecyl vinyl ether, and 380 g of Isopar H was heated to 65° C. with stirring under nitrogen gas stream and, after adding 1.5 g of A.I.V.N. to the reaction mixture, the reaction was carried out for 4 hours. After cooling, the reaction mixture was passed through a 200 mesh nylon cloth to obtain the desired latex grains having a mean grain size of 0.28  $\mu\text{m}$  as a white dispersion.

**PRODUCTION EXAMPLE 104 OF LATEX  
GRAINS: D-104**

A mixed solution of 20 g of the dispersion-stabilizing resin P-13 and 470 g of n-dodecane was heated to 60° C. with stirring under nitrogen gas stream. Then, to the solution was added dropwise a mixed solution of 100 g of methyl methacrylate, 1.0 g of n-dodecylmercaptan and 0.8 g of A.I.V.N. over 2 hours. After reacting for 2 hours, 0.3 g of A.I.V.N. was added to the mixture, followed by reacting for 2 hours. After cooling, the reaction mixture was passed through a 200 mesh nylon cloth in order to remove coarse grains to obtain the desired latex grains having a mean grain size of 0.25  $\mu\text{m}$  as a white dispersion.

**PRODUCTION EXAMPLE 105 OF LATEX  
GRAINS: D-105**

A mixed solution of 14 g of the dispersion-stabilizing resin P-16, 100 g of vinyl acetate, 5 g of crotonic acid, 1.5 g of oxadecyl methacrylate and 468 g of Isopar E was heated to 70° C. with stirring under nitrogen gas stream and, after adding 0.8 g of A.I.V.N., the mixture was reacted for 6 hours. After elevating the temperature to 100° C., the mixture was stirred for 1 hour, and the remaining vinyl acetate was distilled off. After cooling, the reaction mixture was passed through a 200 mesh nylon cloth in order to remove coarse grains to obtain the desired latex grains having a mean grain size of 0.24  $\mu\text{m}$  with a polymerization ratio of 85% as a white dispersion.

**PRODUCTION EXAMPLE 106 OF LATEX  
GRAINS: D-106**

A mixed solution of 15 g of the dispersion-stabilizing resin P-13, 100 g of vinyl acetate, 6.0 g of 4-pentanoic acid and 380 g of Isopar G was heated to 75° C. with stirring under nitrogen gas stream and, after adding 0.7 g of A.I.V.N., the mixture was reacted for 4 hours and, after further adding thereto 0.5 g of A.I.V.N., the reaction was carried out for 2 hours. After cooling, the reaction mixture was passed through a 200 mesh nylon cloth so as to remove coarse grains to obtain the desired latex grains having a mean grain size of 0.23  $\mu\text{m}$  as a white dispersion.

**PRODUCTION EXAMPLE 107 OF LATEX  
GRAINS: COMPARATIVE EXAMPLE E**

By following the same procedure as Production Example 75 of latex grains D-75 except that a mixed solution of 20 g of poly(octadecyl methacrylate), 100 g of vinyl acetate, 1 g of octadecyl methacrylate, and 385 g of Isopar H was used in place of the mixture used in Production Example 75, latex grains having a mean grain size of 0.20  $\mu\text{m}$  were obtained with a polymerization ratio of 85% as a white dispersion. (Latex grains disclosed in JP-A-60-179751)

**PRODUCTION EXAMPLE 108 OF LATEX  
GRAINS: COMPARATIVE EXAMPLE F**

By following the same procedure as Production Example 75 of latex grains D-75 except that a mixed solution of 10 g of the dispersion-stabilizing resin R-1 used in Comparative Example B, 100 g of vinyl acetate, 1 g of Monomer (I) used in Comparative Example B and 385 g of Isopar H was used in place of the mixture used in Production Example 75, latex grains having a mean grain size of 0.24  $\mu\text{m}$  were obtained with a polymerization ratio of 86% as a white dispersion. (Latex grains disclosed in JP-A-61-63855)

**EXAMPLE 1**

In a paint shaker (manufactured by Tokyo Seiki K.K.) were placed 10 g of a dodecyl methacrylate/acrylic acid copolymer (95/5 by weight ratio), 10 g of nigrosine, and 30 g of Shellsol 71 together with glass beads and they were dispersed for 4 hours to obtain a fine dispersion of nigrosine.

Then, a liquid developer for electrostatic photography was prepared by diluting 30 g of the latex grains D-1 obtained in Production Example 1 of latex grains, 2.5 g of the above-prepared nigrosine dispersion, 15 g of a higher alcohol, FOC-1400 (trade name, made by Nissan Chemical Industries, Ltd.) and 0.08 g of an octadecene-octadecylamide semi-maleate copolymer diluted with one liter of Shellsol 71.

**COMPARATIVE LIQUID DEVELOPERS A AND B**

Two kinds of comparative liquid developers A and B were prepared in the same manner as above except that each of the following resin dispersions (latex grains) was used in place of the latex grains D-1 used above.

**COMPARATIVE LIQUID DEVELOPER A**

The latex grains obtained in Production Example 25 of latex grains.

**Comparative Liquid Developer B**

The latex grains obtained in Production Example 26 of latex grains.

An electrophotographic light-sensitive material, ELP Master II Type (trade name, made by Fuji Photo Film Co., Ltd.) was image-exposed and developed by a full-automatic plate-making machine, ELP 404V (trade name, made by Fuji Photo Film Co., Ltd.) using each of the liquid developers thus prepared. The processing (plate-making) speed was 5 plates/minute. Furthermore, after processing 2,000 plates of ELP master II Type, the occurrence of stains of the developing apparatus by sticking of the toner was observed. The blackened ratio (imaged area) of the duplicated images was determined using 30% original. The results obtained are shown in Table 8 below.

**TABLE 8**

| Test No. | Liquid Developer        | Stains of                       |                                                                                 | Image of the 2,000th Plate | Printing Durability     | Remarks             |
|----------|-------------------------|---------------------------------|---------------------------------------------------------------------------------|----------------------------|-------------------------|---------------------|
|          |                         | Developing Apparatus            | Image of the 2,000th Plate                                                      |                            |                         |                     |
| 1        | Developer of Example 1  | No toner residue adhered.       | Clear                                                                           |                            | More than 10,000 sheets | Invention           |
| 2        | Comparative Developer A | Toner residue slightly adhered. | Letter part lost, density of solid black lowered.<br>background portion fogged. | 6,000 sheets               |                         | Comparative Example |
| 3        | Comparative             | Toner residue adhered.          | Fine lines slightly blurred.                                                    | 8,000 sheets               |                         | Comparative Example |

TABLE 8-continued

| Test No. | Liquid Developer | Stains of Developing Apparatus | Image of the 2,000th Plate | Printing Durability | Remarks |
|----------|------------------|--------------------------------|----------------------------|---------------------|---------|
|          | Developer B      |                                | Dmax decreased.            |                     |         |

As is clear from the results shown in Table 8, when printing plates were produced by the above-described processing condition using each liquid developer, only 10 the liquid developer of the present invention caused no stains of the developing apparatus and showed clear images of the 2,000th plate.

Then, the offset printing master plate (ELP Master) prepared using each of the liquid developers was used 15 for printing in a conventional manner, and the number of prints obtained before the occurrences of defects of letters on the images of the prints, the blur of solid black portions, etc., was checked. The results showed that the master plate obtained by using the liquid developer of 20 the present invention provided more than 10,000 prints without accompanied by the above-described failures, whereas the master plates obtained by using the liquid developers of Comparative Examples A and B showed the above-described failures on 6,000 prints and 8,000 25 prints, respectively.

As is clear from the above results, only the liquid developer according to the present invention could advantageously used for preparing a large number of prints by the master plate without causing stains on the 30 developing apparatus by sticking of the toner.

When the liquid developers of Comparative Examples A and B were used under severe plate-making conditions (usually, the blackened ratio of the reproduced image at a plate making speed of 2 to 3 plates per 35 minute is about 8 to 10%), stains on the developing apparatus occurred, in particular, on the back surface of electrodes, and, after developing about 2,000 plates, the image quality of the reproduced image on the plate became to be adversely affected (e.g., decrease in 40 Dmax, blurring of fine lines, etc.). Also, in Comparative Example A, the number of prints obtained by the master plate was markedly decreased.

The above results indicate that the resin grains according to the present invention are clearly excellent as 45 compared with the comparative resins.

#### EXAMPLE 2

A mixture of the white resin dispersion obtained in Production Example 2 of latex grains and 1.5 g of 50 Sumikalon black was heated to 100° C. and stirred for 4 hours at the temperature. After cooling to room temperature, the reaction mixture was passed through a 200 mesh nylon cloth to remove the remaining dye, whereby a black resin dispersion having a mean grain 55 size of 0.24  $\mu$ m was obtained.

Then, a liquid developer was prepared by diluting 32 g of the above-prepared black resin dispersion, 0.05 g of 55 zirconium naphthenate, and 20 g of a higher alcohol, FOC-1600 (trade name, made by Nissan Chemical Industries, Ltd.) with one liter of Shellsol 71.

When the liquid developer was applied to the same developing apparatus as in Example 1 for making printing plates, no occurrence of stains of the developing apparatus by sticking of the toner was observed even 60 after developing 2,000 plates.

Also, the quantity of the offset printing master plate obtained was clear and also the image quality of the

10,000 prints formed using the master plate was very clear.

#### EXAMPLE 3

A mixture of 100 g of the white dispersion obtained in Production Example 22 of latex grains and 3 g of Victoria Blue B was heated to a temperature of from 70° C. to 80° C. with stirring for 6 hours. After cooling to room temperature, the reaction mixture was passed through a 200 mesh nylon cloth to remove the remaining dye, thereby a blue resin dispersion having a mean grain size of 0.23  $\mu$ m was obtained.

Then, a liquid developer was prepared by diluting 32 g of the above-prepared blue resin dispersion, and 0.05 g of zirconium naphthenate with one liter of Isopar H.

When the liquid developer was applied to the same developing apparatus as in Example 1 for making printing plates, no occurrence of stains of the developing apparatus by sticking of the toner was observed even after developing 2,000 plates. Also, the image quality of the images on the offset printing master plate obtained was clear and also the image quality of the 10,000th print was very clear.

#### EXAMPLE 4

A liquid developer was prepared by diluting 32 g of the white dispersion obtained in Production Example 6 of latex grains, 2.5 g of the above-prepared nigrosine dispersion obtained in Example 1, 20 g of FOC-1400 (trade name, made by Nissan Chemical Industries, Ltd.) and 0.02 g of a semi-docosanylamidated compound of a diisobutylene/maleic anhydride copolymer with one liter of Isopar G.

When the liquid developer was applied to the same developing apparatus as in Example 1 for making printing plates, no occurrence of stains of the developing apparatus by sticking of the toner was observed even after developing 2,000 plates. Also, the image quality of the images on the offset printing master plate obtained was clear and also the image quality of the 10,000th print was very clear.

Furthermore, when the liquid developer was allowed to stand for 3 months and then the same processing as above was performed using the developer, the results were the same as those of the developer before storage.

#### EXAMPLE 5

In a paint shaker were placed 10 g of poly(decyl methacrylate), 30 g of Isopar H, and 8 g of Alkali Blue together with glass beads followed by dispersing them for 2 hours to obtain a fine dispersion of Alkali Blue.

Then, a liquid developer was prepared by diluting 30 g of the white resin dispersion D-5 obtained in Production Example 5 of latex grains, 4.2 g of the above-prepared Alkali Blue dispersion, 15 g of isostearyl alcohol, and 0.06 g of a semi-docosanylamidated compound of a copolymer of diisobutylene and maleic anhydride with one liter of Isopar G.

When the liquid developer was applied to the same developing apparatus as in Example 1 for making printing plates, no occurrence of stains of the developing apparatus by sticking of the toner was observed even

after developing 2,000 plates. Also, the image quality of the images on the offset printing master plate and the images of the 10,000th print was very clear.

#### EXAMPLES 6 TO 21

By following the same procedure as Example 5 except that each of the latex grains shown in Table 9 below was used in place of the white resin dispersion D-5, each of liquid developers of was prepared.

TABLE 9

| Example No. | Latex Grains |
|-------------|--------------|
| 6           | D-1          |
| 7           | D-2          |
| 8           | D-3          |
| 9           | D-5          |
| 10          | D-7          |
| 11          | D-8          |
| 12          | D-16         |
| 13          | D-11         |
| 14          | D-12         |
| 15          | D-13         |
| 16          | D-15         |
| 17          | D-16         |
| 18          | D-17         |
| 19          | D-18         |

TABLE 10

| Test No. | Liquid Developer        | Stains of Developing Apparatus | Image of the 2,000th Plate                                                   | Remarks               |
|----------|-------------------------|--------------------------------|------------------------------------------------------------------------------|-----------------------|
| 5        | Developer of Example 22 | No toner residue adhered.      | Clear                                                                        | Invention             |
| 6        | Comparative Developer C | Toner residue greatly adhered. | Letter part lost, density of solid black lowered, background portion fogged. | Comparative Example C |
| 7        | Comparative Developer D | Toner residue adhered.         | Fine lines slightly blurred. Dmax decreased.                                 | Comparative Example D |
| 20       |                         | D-19                           |                                                                              |                       |
| 21       |                         | D-10                           |                                                                              |                       |

When each liquid developer was applied to the same developing apparatus as in Example 1 for making printing plates, no occurrence of stains of the developing apparatus by sticking of the toner was observed even after developing 2,000 plates. Also, the image quality of each offset printing master plate observed and the images of the 10,000th print were very clear.

Furthermore, when the liquid developer was allowed to stand for 3 months and then the same processing as above was performed using the developer, the results were the same as those of the developer before storage.

#### EXAMPLE 22

In a paint shaker (manufactured by Tokyo Seiki K.K.) were placed 10 g of a copolymer of dodecyl methacrylate/acrylic acid copolymer (95/5 by weight ratio), 10 g of nigrosine, and 30 g of Shellsol 71 together with glass beads followed by dispersing for 4 hours to obtain a fine dispersion of nigrosine.

Then, a liquid developer for electrostatic photography was prepared by diluting 30 g of the resin dispersion obtained in Production Example 27 of latex grains, 2.5 g of the above-prepared nigrosine dispersion, 15 g of FOC-1400 (trade name of tetradecyl alcohol, made by Nissan Chemical Industries, Ltd.) and 0.08 g of a copolymer of octadecene and octadecylamide semimaleate, with one liter of Shellsol 71.

#### COMPARATIVE LIQUID DEVELOPERS C AND D

Two kinds of comparative liquid developers C and D were prepared by following the procedure described in

Example 22 but using each of the following resin dispersions in place of the resin dispersion used above.

#### Comparative Liquid Developer C

5 The latex grains obtained in Production Example 73 of latex grains.

#### Comparative Liquid Developer D

The latex grains obtained in Production Example 74 of latex grains.

An electrophotographic light-sensitive material, ELP Master II Type (trade name, made by Fuji Photo Film Co., Ltd.) was imagewise-exposed and developed by a full-automatic plate-making machine, ELP 560 (trade name, made by Fuji Photo Film Co., Ltd.) using each of the liquid developers. The processing (plate-making) speed was 5 plates/minute. Furthermore, the occurrence of stains of the developing apparatus by sticking of the toners after processing 2,000 plates of ELP Master II Type was checked. The blackened ratio (imaged area) of the duplicated images was determined using 30% original. The results obtained are shown in Table 10 below.

TABLE 10

| Test No. | Liquid Developer        | Stains of Developing Apparatus | Image of the 2,000th Plate                                                   | Remarks               |
|----------|-------------------------|--------------------------------|------------------------------------------------------------------------------|-----------------------|
| 5        | Developer of Example 22 | No toner residue adhered.      | Clear                                                                        | Invention             |
| 6        | Comparative Developer C | Toner residue greatly adhered. | Letter part lost, density of solid black lowered, background portion fogged. | Comparative Example C |
| 7        | Comparative Developer D | Toner residue adhered.         | Fine lines slightly blurred. Dmax decreased.                                 | Comparative Example D |

35 As is clear from the results shown in Table 10, when printing plates were produced by the above-described processing condition using each liquid developer, only the liquid developer of the present invention caused no staining of the developing apparatus and gave clear images of the 2,000th plate.

Then, the offset printing master plate (ELP Master) prepared using each liquid developer was used for printing in a conventional manner, and the number of prints obtained before the occurrences of defects of letters on the images of the prints, the blur of solid black portions, etc., was checked. The results showed that the master plate obtained by using each of the liquid developer of the present invention and the comparative liquid developers C and D provided more than 10,000 prints without accompanied by the above-described failures.

As is clear from the above results, only the liquid developer according to the invention could advantageously used for preparing a large number of prints by the master plate without causing stains on the developing apparatus by sticking of the toner.

When the liquid developers of Comparative Examples C and D were used under severe plate-making conditions (usually, the blackened ratio of the reproduced image at a plate-making speed of 2 to 3 plates per minute is about 8 to 10%), stains on the developing apparatus occurred, in particular, on the back surface of electrodes, and, after developing about 2,000 plates, the image quality of the reproduced image on the plate became to be adversely affected (e.g., decrease in Dmax, blurring of fine lines, etc.). Accordingly, these master plates were not practically useful due to deteriorated image quality of prints from the beginning of the printing.

The above results indicate that the resin grains according to the present invention are clearly excellent as compared with the comparative resins.

#### EXAMPLE 23

A mixture of 100 g of the white resin dispersion (D-18) obtained in Production Example 28 of latex grains and 1.5 g of Sumikaron Black was heated to 100° C. and stirred for 4 hours at that temperature. After cooling to room temperature, the reaction mixture was passed through a 200 mesh nylon cloth to remove the remaining dye, whereby a black resin dispersion having a mean grain size of 0.24  $\mu\text{m}$  was obtained.

Then, a liquid developer was prepared by diluting 32 g of the above-described black resin dispersion, 0.05 g of zirconium naphthenate, and 20 g of hexadecyl alcohol, FOC-1600 (made by Nissan Chemical Industries, Ltd.) with one liter of Shellsol 71.

When the liquid developer was applied to the same developing apparatus as in Example 12 for making printing plates, no occurrence of stains of the developing apparatus by sticking of the toner was observed even after developing 2,000 plates.

Also, the image quantity of the offset printing master plate obtained was clear and the images of the 10,000th print were very clear.

#### EXAMPLE 24

A mixture of 100 g of the white resin dispersion (D-70) obtained in Production Example 70 of latex grains and 3 g of Victoria Blue B was heated to a temperature of from 70° C. to 80° C. followed by stirring for 6 hours. After cooling to room temperature, the reaction mixture was passed through a 200 mesh nylon cloth to remove the remaining dye, whereby a blue resin dispersion having a mean grain size of 0.25  $\mu\text{m}$  was obtained.

Then, a liquid developer was prepared by diluting 32 g of the above-described blue resin dispersion, and 0.05 g of zirconium naphthenate with one liter of Isopar H.

When the liquid developer was applied to the same developing apparatus as in Example 22 for making printing plates, no occurrence of stains of the developing apparatus by sticking of the toner was observed even after developing 2,000 plates.

Also, the images of the offset printing master plate obtained were clear, and the images of the 10,000th print were very clear.

#### EXAMPLE 25

A liquid developer was prepared by diluting 32 g of the white resin dispersion (D-32) obtained in Production Example 32 of latex grains, 2.5 g of the nigrosine dispersion prepared in Example 22, 20 g of tetradecyl alcohol, FOC-1400 (made by Nissan Chemical Industries, Ltd.) and 0.02 g of a semi-docosanyl amide compound of a copolymer of diisobutylene and maleic anhydride with one liter of Isopar G.

When the liquid developer was applied to the same developing apparatus as in Example 22 for making printing plates, no occurrence of stains of the developing apparatus by sticking of the toner was observed even after developing 2,000 plates.

Also, the image quality of the offset printing master plate obtained were clear and the images of the 10,000th print were very clear.

Furthermore, when the liquid developer was allowed to stand for 3 months and then used for the same pro-

cessing as above, the results obtained were almost the same as above.

#### EXAMPLE 26

In a paint shaker were placed 10 g of poly(decyl methacrylate), 30 g of Isopar H, and 8 g of Alkali Blue together with glass beads followed by dispersing them for 2 hours to prepare a fine dispersion of Alkali Blue.

Then, a liquid developer was prepared by diluting 30 g of the white resin dispersion (D-31) obtained in Production Example 31 of latex grains, 4.2 g of the above-prepared Alkali Blue, 15 g of isostearyl alcohol, and 0.06 g of a semi-docosanyl amide compound of a copolymer of diisobutylene and maleic anhydride with one liter of Isopar G.

When the liquid developer was applied to the same developing apparatus as in Example 22 for making printing plates, no occurrence of stains of the developing apparatus by sticking of the toner was observed even after developing 2,000 plates. Also, the image quality of the images on the offset master plate and images of the 10,000th print were very clear.

#### EXAMPLES 27 TO 46

By following the same procedure as Example 26 except that each of the latex grains shown in Table 11 was used in place of the white resin dispersion (D-31) produced in Production Example 31 of latex grains, each of liquid developers was prepared.

TABLE 11

| Example No. | Latex Grains |
|-------------|--------------|
| 27          | D-27         |
| 28          | D-28         |
| 29          | D-29         |
| 30          | D-30         |
| 31          | D-32         |
| 32          | D-33         |
| 33          | D-34         |
| 34          | D-35         |
| 35          | D-36         |
| 36          | D-37         |
| 37          | D-38         |
| 38          | D-39         |
| 39          | D-42         |
| 40          | D-46         |
| 41          | D-47         |
| 42          | D-50         |
| 43          | D-51         |
| 44          | D-53         |
| 45          | D-54         |
| 46          | D-56         |

When each of the liquid developer was applied to the developing apparatus as in Example 22, no occurrence of stains of the developing apparatus by sticking of the toner was observed even after developing 2,000 plates.

Also, the image quality of each offset printing master plate obtained and the images of the 10,000th prints obtained in each case were very clear.

Furthermore, when the liquid developer was allowed to stand for 3 months and then used for the same processing as above, the results obtained were almost the same as above.

#### EXAMPLE 47

In a paint shaker (manufactured by Tokyo Seiki K.K.) were placed 10 g of a dodecyl methacrylate/acrylic acid copolymer (95/5 by weight ratio), 10 g of nigrosine, and 30 g of Shellsol 71 together with glass

beads followed by dispersing for 4 hours to obtain a fine dispersion of nigrosine.

Then, a liquid developer was prepared by diluting 30 g of the resin dispersion (D-75) produced in Production Example 75 of latex grains, 2.5 g of the above-prepared nigrosine dispersion, 15 g of tetradecyl alcohol, FOC-1400 (made by Nissan Chemical Industries, Ltd.) and 0.08 g of a copolymer of octadecene and octadecylamine semi-maleate with one liter of Shellsol 71.

#### COMPARATIVE LIQUID DEVELOPERS E AND F

Two kinds of comparative liquid developers E and F were prepared in the same manner as in Example 47 except that each of the following resin dispersions (latex grains) was used in place of the above resin dispersion.

##### Comparative Liquid Developer E

The resin dispersion obtained in Production Example 107 of latex grains.

##### Comparative Liquid Developer F

The resin dispersion obtained in Production Example 108 of latex grains.

The resulting liquid developers were evaluated in the same manner as in Example 22, and the results obtained are shown in Table 12 below.

TABLE 12

| Example No.           | Liquid Developer        | Stains of Developing Apparatus  | Image of the 2,000th Plate                                                   | Printing Durability     |
|-----------------------|-------------------------|---------------------------------|------------------------------------------------------------------------------|-------------------------|
| Example 47            | Developer of Example 47 | No toner residue adhered.       | Clear                                                                        | more than 10,000 sheets |
| Comparative Example E | Comparative Developer E | Toner residue markedly adhered. | Letter part lost, density of solid black lowered, background portion fogged. | 8,000 sheets            |
| Comparative Example F | Comparative Developer F | Toner residue adhered.          | Fine lines slightly blurred. Dmax decreased.                                 | 8,000 sheets            |

As is clear from the results shown in Table 12, when printing plates were produced by the above-described processing condition using each liquid developer, the only liquid developer of the present invention caused no stains of the developing apparatus and gave the 2,000th printing plate having clear images.

Then, the offset printing master plate (ELP Master) prepared using each liquid developer was used for printing in a conventional manner, and the number of prints obtained before the occurrences of defects of letters on the images of the prints, the blur of solid black portions, etc., was checked. The results showed that the master plate obtained using the liquid developer of the present invention provided more than 10,000 prints without accompanied by the above-described failures, whereas the master plates obtained by using the liquid developers of Comparative Examples E and F showed the above-described failures on 8,000 prints.

As is clear from the above results, the only liquid developer according to the present invention could advantageously used for preparing a large number of prints by the master plate without causing stains on the developing apparatus by sticking of the toner.

When the liquid developers of Comparative Examples E and F were used under severe plate-making conditions (usually, the blackened ratio of the reproduced image at a plate-making speed of 2 to 3 plates per minutes is about 8 to 10%), stains on the developing apparatus occurred, in particular, on the back surface of electrodes, and, after developing about 2,000 plates, the image quality of the reproduced image on the plate

became to be adversely affected (e.g., decrease in Dmax, blurring of fine lines, etc.).

The above results indicate that the resin grains according to the present invention are clearly excellent as compared with the comparative resins.

#### EXAMPLE 48

A mixture of 100 g of the white resin dispersion D-76 obtained in Production Example 76 of latex grains and

10 1.5 g of Sumikalon Black was heated to 100° C. followed by stirring for 4 hours. After cooling, the reaction mixture was passed through a 200 mesh nylon cloth to remove the remaining dye, whereby a black resin dispersion having a mean grain size of 0.24  $\mu\text{m}$  was obtained.

Then, a liquid developer was prepared by diluting 32 g of the above-described black resin dispersion, 0.05 g of zirconium naphthenate, and 20 g of FOC-1600 (hexadecyl alcohol made by Nissan Chemical Industries, Ltd.) with one liter of Shellsol 71.

When the resulting liquid developer was applied to the developing apparatus as in Example 22 for making printing plates, no occurrence of stains of the developing apparatus by sticking of the toner was observed even after developing 2,000 plates.

Also, the image quantity of the offset printing master plate obtained was clear and images of the 10,000th

40 prints were very clear.

#### EXAMPLE 49

A mixture of 100 g of the white resin dispersion D-106 obtained in Production Example 106 of latex grains and 3 g of Victoria Blue was heated to a temperature of from 70° C. to 80° C. followed by stirring for 6 hours. After cooling to room temperature, the reaction mixture was passed through a 200 mesh nylon cloth to remove the remaining dye, whereby a blue resin dispersion having a mean grain size of 0.23  $\mu\text{m}$  was obtained.

Then, a liquid developer was prepared by diluting 32 g of the above-described blue resin dispersion, and 0.05 g of zirconium naphthenate with one liter of Isopar H.

When the resulting liquid developer was applied to the developing apparatus as in Example 22, no occurrence of stains of the developing apparatus by sticking of the toner was observed even after developing 2,000 plates.

Also, the image quality of the offset printing master plate obtained was clear and the images of the 10,000th print was clear.

#### EXAMPLE 50

A liquid developer was prepared by diluting 32 g of the white resin dispersion D-80 obtained in Production Example 80 of latex grains, 1.5 g of the nigrosine dispersion obtained in Example 47, 20 g of FOC-1400 (tetradecyl alcohol made by Nissan Chemical Industries,

Ltd.) and 0.02 g of a semi-docosenylamidated compound of an isobutylene/maleic anhydride copolymer with one liter of Isopar G.

When the resulting liquid developer was applied to the developing apparatus as in Example 22, no occurrence of stains of the developing apparatus by sticking of the toner was observed even after developing 2,000 plates.

Also, the image quality of the offset printing master plate obtained was clear and the images of the 10,000th print were clear.

Furthermore, when the liquid developer was allowed to stand for 3 months and used for the processing as above, the results obtained were almost the same as above.

#### EXAMPLE 51

In a paint shaker were placed 10 g of poly(decyl methacrylate), 30 g of Isopar H, and 8 g of Alkali Blue together with glass beads followed by dispersing for 2 hours to prepare a fine dispersion of Alkali Blue.

Then, a liquid developer was prepared by diluting 30 g of the white resin dispersion D-79 obtained in Production Example 79 of latex grains, 4.2 g of the above-prepared Alkali Blue dispersion, 15 g of FOC-1400 (isostearyl alcohol made by Nissan Chemical Industries, Ltd.), and 0.06 g of a semi-docosenylamidated product of a copolymer of diisobutylene and maleic anhydride with one liter of Isopar G.

When the liquid developer was applied to the developing apparatus as in Example 22 for making printing plates, no occurrence of stains of the developing apparatus by sticking of the toner was observed even after developing 2,000 plates.

Also, the image quality of the offset printing master plate obtained and the images of the 10,000th print was very clear.

#### EXAMPLES 52 TO 57

By following the same procedure as Example 51 except that each of the latex grains shown in Table 13 below was used in place of the white resin dispersion D-79 obtained in Production Example 79 of latex grains, each of liquid developers was prepared.

TABLE 13

| Example No. | Latex Grains |
|-------------|--------------|
| 52          | D-75         |
| 53          | D-76         |
| 54          | D-77         |
| 55          | D-81         |
| 56          | D-85         |
| 57          | D-87         |

When each of the liquid developer was applied to the same developing apparatus as in Example 22 for making printing plates, no occurrence of stains of the developing apparatus by sticking of the toner was observed even after developing 2,000 plates.

Also, the image quality of the offset printing master plate obtained and the images of the 10,000th print were very clear.

Furthermore, when the liquid developer was allowed to stand for 3 months and used for the processing as above, the results obtained were almost the same as above.

While the invention has been described in detail and with reference to specific embodiments thereof, it will be apparent to one skilled in the art that various changes

and modifications can be made therein without departing from the spirit and scope thereof.

What is claimed is:

1. A liquid developer for electrostatic photography comprising at least resin grains dispersed in a non-aqueous solvent having an electric resistance of at least  $10^9 \Omega\text{cm}$  and a dielectric constant of not higher than 3.5, wherein the dispersed resin grains are polymer resin grains obtained by polymerizing a solution containing at least one mono-functional monomer (A) which is soluble in said non-aqueous solvent but becomes insoluble therein by being polymerized, in the presence of a dispersion-stabilizing resin which is soluble in said non-aqueous solvent and which is a graft type copolymer formed from (1) at least one mono-functional macromonomer (M) having a weight average molecular weight of from  $1 \times 10^3$  to  $2 \times 10^4$  comprising an AB block copolymer having a polymerizable double bond bonded to the terminal of the polymer main chain of the B block of said AB block copolymer, and (2) at least one monomer (B) represented by the following general formula (II), said AB block copolymer being composed of an A block comprising a polymer component containing at least one polar group selected from a phosphono group, a carboxy group, sulfo group, a hydroxyl group, a formyl group, a carboxyamido group, a sulfoamide group, an amino group, and a



group (wherein  $\text{R}_{11}$  represents  $-\text{R}_{12}$  or  $-\text{OR}_{12}$  (wherein  $\text{R}_{12}$  represents a hydrocarbon group)) and/or a polymer component corresponding to the mono-functional monomer (A) and a B block containing at least one polymer component represented by the following general formula (I):



wherein  $\text{V}_0$  represents  $-\text{COO}-$ ,  $-\text{OCO}-$ ,  $-\text{CH}_2-$ ,  $-\text{OCO}-\text{CH}_2-\text{COO}-$  (wherein  $\text{l}_1$  and  $\text{l}_2$  each represents an integer of from 1 to 3),  $-\text{O}-$ ,  $-\text{SO}_2-$ ,  $-\text{CO}-$ ,



$\text{CONHCOO}-$ ,  $-\text{CONHCONH}-$  or



(wherein  $\text{R}_{13}$  represents a hydrogen atom or a hydrocarbon group),  $\text{R}_0$  represents a hydrocarbon group, and  $\text{a}_1$  and  $\text{a}_2$ , which may be the same or different, each represents a hydrogen atom, a halogen atom, a cyano group, a hydrocarbon group having from 1 to 8 carbon atoms,  $-\text{COO}-\text{Z}_1$  or  $-\text{COO}-\text{Z}_1$  bonded via a hydro-

carbon group (wherein  $Z_1$  represents a hydrocarbon group having from 1 to 22 carbon atoms):



(II)

wherein  $V_1$  represents  $-\text{COO}-$ ,  $-\text{OCO}-$ ,  $-\text{CH}_2-$ ,  $\text{OCO}-$ ,  $-\text{CH}_2-$ ,  $\text{OCO}-$  (wherein  $l_3$  and  $l_4$  each represents an integer of from 1 to 3) or  $-\text{O}-$ ,  $R_1$  represents an aliphatic group having 8 or more carbon atoms, and  $b_1$  and  $b_2$ , which may be the same or different, each represents a hydrogen atom, a halogen atom or a hydrocarbon group having from 1 to 6 carbon atoms.

2. The liquid developer for electrostatic photography as in claim 1, wherein the dispersed resin grains are copolymer resin grains obtained by polymerizing a solution containing at least one mono-functional monomer (A) which is soluble in the non-aqueous solvent but becomes insoluble therein by being polymerized and at least one monomer (C) represented by following formula (III), said monomer (C) having at least two polar groups and/or polar linking groups:



(III)

wherein  $U_1$  represents  $-\text{O}-$ ,  $-\text{COO}-$ ,  $-\text{OCO}-$ ,  
 $-\text{CH}_2\text{OCO}-$ ,  $-\text{SO}_2-$ ,  $-\text{CONH}-$ ,  $-\text{SO}_2\text{NH}-$ ,



(wherein  $E_1$  represents a hydrocarbon group or has the same meaning as the linking group  $A_1-B_1$ ,  $A_2-B_2$ ,  $\rightarrow E_0$  in the formula (III),  $E_0$  represents a hydrogen atom or a hydrocarbon group having from 1 to 18 carbon atoms, which may be substituted with a halogen atom,  $-OH$ ,  $-CN$ ,  $-NH_2$ ,  $-COOH$ ,  $-SO_3H$ , or  $-PO_3H_2$ ;  $B_1$  and  $B_2$ , which may be the same or different, each represents  $-O-$ ,  $-S-$ ,  $-CO-$ ,  $-CO_2-$ ,  $-OCO-$ ,  $-SO_2-$ ,



—NHCO<sub>2</sub>— or —NHCONH— (wherein E<sub>2</sub> has the same meaning as E<sub>0</sub> described above); A<sub>1</sub> and A<sub>2</sub>, which may be the same or different, each represents a hydrocarbon group having from 1 to 18 carbon atoms which may be substituted or may contain



(wherein  $B_3$  and  $B_4$ , which may be the same or different, have the same meaning as  $B_1$  and  $B_2$  described above;  $A_4$  represents a hydrocarbon group having from 1 to 18 carbon atoms, which may be substituted; and  $E_3$  has the same meaning as  $E_0$ ) in the main chain bond;  $d_1$  and  $d_2$ , which may be the same or different, each represents a hydrogen atom, a hydrocarbon group,  $—COO—E_4$  or  $—COO—E_4$  bonded via a hydrocarbon group (wherein

70

E<sub>4</sub> represents a hydrogen atom or a hydrocarbon group which may be substituted); and r, s and t, which may be the same or different, each represents an integer of from 0 to 4, provided that r, s and t cannot be 0 at the same time, in the presence of said dispersion-stabilizing resin.

3. The liquid developer for electrostatic photography as in claim 1, wherein the dispersed resin grains are copolymer resin grains obtained by polymerizing a solution containing at least one mono-functional monomer (A) which is soluble in the non-aqueous solvent but becomes insoluble therein by being polymerized and at least one monomer (D) represented by following formula (IV), said monomer (D) having an aliphatic group having at least 8 carbon atoms and forming a copolymer by the polymerization reaction with said monomer (A);



(IV)

wherein  $E_7$  represents an aliphatic group having at least 8 carbon atoms;  $U_2$  represents  $-\text{COO}-$ ,  $-\text{CONH}-$



(wherein  $E_8$  represents an aliphatic group),  $—OCO—$ ,  $—CH_2COO—$ , or  $—O—$ ; and  $e_1$  and  $e_2$ , which may be the same or different, each represents a hydrogen atom, an alkyl group,  $—COOE_9$ , or  $—CH_2COOE_9$  (wherein  $E_9$  represents an aliphatic group), in the presence of said dispersion-stabilizing resin.

4. The liquid developer for electrostatic photography as in claim 1, wherein said mono-functional monomer (A) is represented by the formula (V):



(V)

wherein  $U_3$  represents  $-\text{COO}-$ ,  $-\text{OCO}-$ ,  $-\text{CH}_2\text{OCO}-$ ,  $-\text{CH}_2\text{COO}-$ ,  $-\text{O}-$ ,  $-\text{CONHCOO}-$ ,  $-\text{CONHOOCO}-$ ,  $-\text{SO}_2-$ .



(wherein  $D_2$  represents a hydrogen atom or an aliphatic group having from 1 to 8 carbon atoms which may be substituted),  $D_1$  represents an aliphatic group having from 1 to 6 carbon atoms which may be substituted, and  $f_1$  and  $f_2$ , which may be the same or different, each represents a hydrogen atom, a halogen atom, a cyano group, a hydrocarbon group having from 1 to 8 carbon atoms,  $-\text{COO}-Z_1$  or  $-\text{COO}-Z_1$  bonded via a hydrocarbon group (wherein  $Z_1$  represents a hydrogen atom or a hydrocarbon group having 1 to 22 carbon atoms).

5. The liquid developer for electrostatic photography as in claim 1, wherein the proportion of the A block to

the B block in said AB block copolymer is from 1 to 50/99 to 50 by weight.

6. The liquid developer for electrostatic photography as in claim 1, wherein said graft type copolymer has a weight average molecular weight of from  $1.5 \times 10^4$  to  $3 \times 10^5$ .

7. The liquid developer for electrostatic photography

as in claim 1, wherein the content of the monomer (B) represented by the formula (II) in said graft type copolymer is from 40 to 99% by weight.

8. The liquid developer for electrostatic photography as in claim 1, wherein said liquid developer contains a colorant.

\* \* \* \* \*

10

15

20

25

30

35

40

45

50

55

60

65